# EUROPEAN PATENT SPECIFICATION

(11) **EP 0 243 866 B1**
(45) Date of publication and mention of the grant of the patent: **09.03.1994**
(21) Application number: 87105906.9
(22) Date of filing: 22.04.1987
(51) Int. Cl.: G03C 7/42

(54) **Method for processing light-sensitive halide color photographic material**
Verfahren zur Behandlung eines lichtempfindlichen farbphotographischen Halogenidmaterials
Méthode de traitement d'un matériau photographique couleur à l'halogénure sensible à la lumière

(30) Priority: 23.04.1986 JP 93917/86; 23.04.1986 JP 93918/86; 10.01.1987 JP 3452/87
(43) Date of publication of application: 04.11.1987
(73) Proprietor: KONICA CORPORATION, Tokyo 163 (JP)
(72) Inventor: Hagiwara nee Higuchi, Moeko, Hino-shi Tokyo (JP); Koboshi, Shigeharu, Hino-shi Tokyo (JP); Kuse, Satoru, Hino-shi Tokyo (JP)
(74) Representative: Gille, Christian, Dipl.-Ing.

(56) References cited:
- EP-A- 0 132 806
- EP-A- 0 143 570
- EP-A- 0 158 369
- EP-A- 0 173 540
- DE-A- 3 518 257
- FR-A- 2 091 025
- FR-A- 2 276 613
- PATENT ABSTRACTS OF JAPAN, vol. 10, no. 300 (P-506)[2356], 14th October 1986; & JP-A-61 117 541
- PATENT ABSTRACTS OF JAPAN, vol. 11, no. 91 (P-558)[2538], 23rd March 1987; & JP-A-61 243 451

## Description

### Background of the invention

This invention relates to a method for processing a light-sensitive silver halide color photographic material. More particularly, it is concerned with a method for processing a light-sensitive silver halide color photographic material without any impairment of recoloring property even if a replenished amount of a bleaching solution is reduced.

From FR-A-2 276 613, JP-A-6 117 541, EP-A-0 143 570 and EP-A-0 158 369 photographic processing methods are known which use bleaching solutions comprising an organic ferric complex and an organic acid. From EP-A-0 158 369 it is further known to replenish the bleaching solutions.

Processing of light-sensitive materials comprises basically two steps of color development and desilvering and the desilvering step comprises a bleaching and fixing steps or a bleach-fixing step. Besides these steps, rinse processing, stabilizing processing and so on may be added as additional processing steps.

In color development, an exposed silver halide is reduced to silver and simultaneously an oxidized aromatic primary amine color developing agent is subjected to reaction with a coupler to form a dye. In this course, the halogen ion produced by development of a silver halide is dissolved into a developing solution and accumulated therein. Also, the components such as a retarder and the like contained in a light-sensitive silver halide photographic material is dissolved into a color developing solution and accumulated therein. In the desilvering step, the silver as produced by development is bleached by an oxidizing agent and then all silver salts are removed from a light-sensitive photographic material as soluble silver salts by a fixing agent.

As a processing solution having a bleaching ability for processing of a light-sensitive silver halide color photographic material, inorganic oxidizing agents such as red prussinate, dichromic acid salts and the like have been widely employed as an oxidizing agent for bleaching of an image silver.

With regard to the processing solution having a bleaching ability and containing such inorganic oxidizing agent, there have been indicated several serious drawbacks. For instance, red prussinate and dichromic acid salts are relatively superior in a bleaching power of image silver, but tend to be decomposed with light to produce a cyan ion and a hexavalent chromium ion, which may be harmful to human beings and show an unfavourable property for prevention of environmental pollution. Additionally, the processing solution containing such inorganic oxidizing agents has a disadvantage of being difficult to regenerate and reuse the waste after processing without discarding.

To the contrary, there has been employed a processing solution containing as an oxidizing agent an organic acid metal complex such as an aminopolycarboxylic acid metal complex and the like for meeting the requirements, e.g., less problem in environmental pollution, rapid processing, simplification and regeneration of waste for reuse. However, the processing solution using the organic acid metal complex has a drawback of a slow bleaching speed (or oxidation speed) of the image silver (metallic silver) formed during developing step due to a slow oxidizing power. For instance, an (ethylenediamine-tetraacetato)iron (III) complex, which is believed to exert a strong bleaching power of aminopolycarboxylic acid metal complexes, has been partially practised as a bleaching solution or a bleach-fixing bath, but it has a drawback of an insufficient bleaching power and a prolonged bleaching step, in a high sensitive light-sensitive silver halide color photographic material containing as a main component a silver bromide or silver iodobromide emulsion, particularly a color paper for photographing, a negative color film for photographing, a color reversal film for photographing and the like, which contain, as a silver halide, silver iodide with a high silver content.

Also, by processing the light-sensitive material as above, a color developing component in previous bath tends to adhere to the light-sensitive material and thereby being brought in and accumulated in a bleaching bath.

Therefore, in a method for continuously developing a large amount of light-sensitive silver halide photographic materials by means of an automatic developing machine, there is required any means for maintaining a given concentration range of components in a processing bath in order to avoid deterioration of performance of a bleaching solution owing to change in component concentrations. As the said means, one has usually adopted a method for repleneishing a replenishing solution to dilute unnecessary increased components and supplement deficient components. By replenishing the replenishing solution, a large volume of overflow tend to be necessarily produced and discarded; this method would pose a great problem economically or in environmental pollution. Accordingly, there have been recently proposed a method wherein such replenishing solutions are condensed and supplied in a small volume in order to decrease the overflowed solution, so-called a condensed, low replenishing system, or another method wherein a regenerating agent is added to the overflowed solution for reuse as a replenishing solution.

With particular respect to a bleaching solution or bath, there has been put to practical use a method wherein the organic acid ferrous complex produced by bleaching a developed silver, e.g., (ethylenediaminetetraacetato)iron (II) complex is oxidized with aeration to (ethylenediaminetetraacetato) iron (III) complex, i.e. the organic acid ferric complex, to which a regenerating agent is then added for supplementing deficient components and the resulting mixture is again used as a replenishing solution.

However, there has appeared recently the so-called compact photofinishing laboratory (also called "miniphoto-finishing laboratory") for processing in a short time and reducing a cost for collection and delivery, where there is a great need for simplification of processing and also for reduction in the area for installing a developing machine and there is not desired a regeneration step required for complicated working and control and also for a processing space.

Therefore, a condensed, low replenishing system is favourable by doing a low replenishing with no regeneration step; an extreme decrease in a replenishing amount of a bleaching solution, however, tends to raise a concentration of color developing components taken into a bleaching solution and to receive the influence by concentration with evaporation more easily, which results in more accumulation of color development components. Thus, when a concentration of color developing components is increased in a bleaching solution, a ratio of contaminating color developing agents as reducing components, sulfites and the like is increased to inhibit bleaching reaction and, more seriously, a color dye, particularly a cyan dye may be easily converted to the corresponding leuco form, whereby there is given a drawback of being insufficient in coloring or readily producing the so-called poor recoloring. This phenomenon may be seen particularly remarkably in a high sensitive light-sensitive material having a high silver level and silver iodide as a main component. Regeneration step is substantially a system for decreasing a replenished amount, but the above-depicted drawback would be difficult to be seen therein, since aeration can be practised, a substantial aeration is effected owing to a prolonged residual time in a stock tank and others except for bleaching tank and a prolonged contact time with air, and a processing time in the prior bleaching step is as long as 6 minutes or longer.

Nevertheless, there has been recently desired a much lower replenishing from demands for lower cost, less environmental pollution and so on. Still further, there has been required even such a service (the so-called 1 Hour Photo) to send back to a user in several hours after received. Under these circumstances, the above-mentioned points have been posing far greater problems.

Also, another problem is that bleaching stain may be produced in a light-sensitive material, when a low replenishing of a bleaching solution is made, owing to increased color developing components accumulated in a bleaching solution as explained hereinabove. It is the actual state that a bleaching stain problem has been more and more actualized, as a photofinishing laboratory with a low processing amount, e.g., recent compact photofinishing laboratory has a poor refreshing rate of a bleaching solution with an increased vaporization volume.

### [Summary of the invention]

It is an object of this invention to provide a method for processing a light-sensitive silver halide color photographic material with a rapid bleaching step and a low replenishment.

Another object of this invention is to provide a method for processing a light-sensitive silver halide color photographic material which shows an excellent silver bleaching efficacy and an improved production of leuco cyan dyes.

A still another object of this invention is to provide a method for processing a light-sensitive silver halide color photographic material with an improved generation of bleaching stain even in a condensed, low replenishing process.

A further object of this invention is to provide a method for processing a light-sensitive silver halide color photographic material with less complicated procedures and less control of processing solutions.

The present inventors have made earnest studies to dissolve the aforesaid problems and found that the aforesaid objects of this invention can be accomplished by a method for processing a light-sensitive silver halide color photographic material having at least one silver halide emulsion layer which comprises subjecting to image-like exposure and subsequently to processing including at least color development step and bleaching step, wherein a bleaching solution employed in said bleaching step contains at least one organic acid ferric complex; and said bleaching solution contains at least one organic acid and said bleaching solution is replenished, characterized in that a light-sensitive silver halide color photographic material is processed wherein at least one layer of said silver halide emulsion layer contains at least one magenta coupler having the general formula (M): wherein Z represents a non-metal atom group necessary to form a nitrogen-containing heterocyclic ring, said ring optionally having a substituent; X represents a hydrogen atom or a substituent eliminable through a reaction with an oxidized product of a color developing agent; and R represents a hydrogen atom or a substituent; that the organic acid is contained in a range of not more than 10 mole % of the content of said organic acid ferric complex contained in said bleaching solution; and that the replenished amount in said bleaching step is 30 m to 300 m per 1m² of said silver halide color photographic material.

As one preferred embodiment of this invention, there is provided the embodiment wherein the bleaching solution in this invention contains at least one of the compounds having the general formulae (I) - (IX) as shown below.

In the formula, Q represents a group of atoms necessary for-the formation of a nitrogen-containing heterocyclic ring (including the ring condensed with an unsaturated 5- to 6-membered ring); and R represents a hydrogen atom, an alkyl group having 1 to 6 carbon atoms, a cycloalkyl group, an aryl group, a heterocyclic ring (including the ring condensed with an unsaturated 5- to 6-membered ring) or an amino group.

In the formula, R₂ and R₃ each represent a hydrogen atom, an alkyl group having 1 to 6 carbon atoms, a hydroxyl group, a carboxyl group, an amino group, an acyl group having 1 to 3 carbon atoms, an aryl group or an alkenyl group.
A represents; or an ni -valent heterocyclic residual group (including the group condensed with an unsaturated 5- to 6- membered ring); X represents = S, = O or = NR". Here, R and R' each have the same meaning as defined for R₂ and R₃; X' has the same meaning as defined for X; Z represents a hydrogen atom, an alkali metal atom, an ammonium group, an amino group, a nitrogen-containing heterocyclic residual group, an alkyl group or M represents a divalent metallic atom; R" represents a hydrogen atom, an alkyl group having 1 to 6 carbon atoms, a cycloalkyl group, an aryl group, a heterocyclic residual group (including the group condensed with an unsaturated 5- to 6-membered ring) or an amino group; and n1 to n6 and m1 to m5 each represent an integer of 1 to 6. B represents an alkylene group having 1 to 6 carbon atoms; Y represents -N 〈 or -CH 〈 ; R₄ and R₅ each have the same meaning as defined for R₂ and R₃; provided that R₄ and R₅ each may represent -B-SZ and that R₂ and R₃, R and R', and R₄ and R₅ each may be combined to form a ring.

The compound represented by the above formula may also include an enol form compound and a salt thereof.

In the formula, R₆ and R₇ each represent a hydrogen atom, an alkyl group having 1 to 6 carbon atoms, a hydroxyl group, a carboxyl group, an amino group, an acyl group having 1 to 3 carbon atoms, an aryl group, an alkenyl group or -B₁-S-Z₁; provided that R₆ and R₇ may be combined to form a ring. Y₁ represents N- or CH-; B represents an alkylene group having 1 to 6 carbon atoms; Z₁ represents a hydrogen atom, an alkali metal atom, an ammonium group, an amino group, a nitrogen-containing heterocyclic residual group or and n7 represents an integer of 1 to 6.

In the formula, R₈ and R₉ each represent or ; and R₁₀ represents an alkyl group or -(CH₂)ₙ₈SO₃⊖ (provided that ℓ represents 0 when R₁₀ is -(CH₂)-ₙ₈SO₃⊖, or 1 when it is an alkyl group). G^{⊖} represents an anion; and n8 represent an integer of 1 to 6.

In the formula, Q₁ represents a group of atoms necessary for the formation of a nitrogen-containing heterocyclic ring (including the ring condensed with an unsaturated or saturated 5- to 6-membered ring); and R₁₁ represents a hydrogen atom, an alkali metal atom, or an alkyl group; provided that Q' have the same meaning as defined for Qi.

In the formula, D₁, D₂, D₃ and D₄ each represent a simple bond arm, an alkylene group having 1 to 8 carbon atoms or a vinylene group; and q1, q2, q3 and q4 each represent an integer of 0, 1 or 2. The ring formed together with a sulfur atom may be further condensed with a saturated or unsaturated 5- to 6- membered ring, with the exception of elementary sulfur;

In the formula, X₂ represents -COOM', -OH, -SO₃M', -CONH₂, -S0₂NH₂, -NH₂, -SH, -CN, -CO₂R₁₆, -SO₂R₁₆, -OR₁₆, -NR₁₆ R₁₇, -SR₁₆, -SO₃ R₁₆, -NHCOR₁₆, -NHS0₂ R₁₆, -OCOR₁₆ or -S0₂ R₁₆; Y₂ represents or a hydrogen atom; and m9 and n9 each represent an integer of 1 to 10. R₁₁, R₁₂, R₁₃, R₁₄, R₁₅, R₁₇ and R₁₈ each represent a hydrogen atom, a lower alkyl group, an acyl group or
R₁₆ represents a lower alkyl group;
R₁₉ represents -NR₂₀R₂₁, -OR₂₂ or -SR₂₂; R₂₀ and R₂₁ each represent a hydrogen atom or a lower alkyl group; and R₂₂ represents a group of atoms necessary for a ring to be formed by combination with R₁₈. R₂₀ or R₁₁ may be combined with R₁₈ to form a ring. M' represents a hydrogen atom or a cation.

In the formula, Ar represents a divalent aryl group or a divalent organic group formed by combination of an aryl group with an oxygen atom and/or alkylene group; B₂ and B₃ each represent a lower alkylene group; R₂₃, R₂₄, R₂₅ and R₂₆ each represent a hydroxyl substituted lower alkyl group; and x and y each represent 0 or 1. G' represents an anion; and z represents 0, 1 or 2.

In the formula, R₂₉ and R₃₀ each represent a hydrogen atom, an alkyl group, an aryl group or a heterocyclic group; R₃, represents a hydrogen atom or an alkyl group; R₃₂ represents a hydrogen atom or a carboxyl group.

The compounds represented respectively by General Formulae (I) to (IX) preferably used in this invention are compounds generally used as bleach accelerators, which are hereinafter referred to as the bleach accelerators of this invention.

Typical examples of the bleach accelerators of this invention may include, for example, the following, but by no means limited to these.

As another preferable embodiment of this invention, there is the embodiment wherein at least one layer of said silver halide color photographic material contain a cyan coupler having the general formula (C). (wherein R₂, represents an alkyl group, an alkenyl group, a cycloalkyl group, an aryl group or a heterocyclic group; R₂₄ represents an unsubstituted or substituted aryl group; and Z represents a hydrogen atom or a group eliminatabile through a coupling reaction with an oxidizing product of a N-hydroxyalkyl substituted-p-phenylenediamine derivative developing agent).

As further preferred embodiment of this invention, there is the embodiment wherein the magenta coupler of formula (M) has at least one aromatic sulfonyl group represented by the following formula in its molecular structure: wherein R represents an aliphatic group, an aryl group or a heterocyclic group; m represents an integer of 1 or 2, R may be identical or different when m is 2; R₂ represents an aliphatic group, an aryl group, a heterocyclic group or when R₃ and R₄ each represent a hydrogen atom, an aliphatic group or an aryl group.

### [Detailed description of the invention]

This invention will be more fully illustrated hereinbelow.

In regeneration of a bleaching solution, a large amount of a free organic acid as a stabilizer has been hithereto incorporated in order to prevent precipitation and decomposition caused by organic acid ferric complex in aeration.

Now, the present inventors have found that the aforesaid object of this invention can be accomplished by keeping a free organic acid concentration in a bleaching solution at a molar percent of not more than 10 mole % to the organic acid ferric complex as a bleaching agent in a light-sensitive material.

In adopting a condensed, low replenishing method, a contact time with air becomes longer due to a prolonged residual time of a bleaching solution in a stock tank and so on or due to enforced aeration, and it has been found that precipitation or decomposition caused by the organic acid ferric complex can be improved even if a substantial aeration is done. Moreover, it is surprising that there can be also reduced the bleaching stain caused by color developing components accumulated in a bleaching solution, i.e. oxidized products of color developing agents.

An amount of the present bleaching solution to be replenished is 30 mî to 300 mℓ per 1 m² of a light-sensitive silver halide color photographic material, more preferably 40 mℓ to 250 mt, most preferably 50 m to 200 mℓ.

The organic acid or organic acid capable of forming the organic acid ferric complex may be suitably an aminocarboxylic acid compound or an amin acid compound, namely the amino compound having at least 2 or more carboxy groups or the amino compound having at least 2 or more phosphonic acid groups; preferably those compounds having the following general formulae (XII) and (XIII).

In the above formulae, E represents a substituted or unsubstituted alkylene group, a cycloalkylene group, a phenylene group, -R₈₃0R₈₃0R₈₃- or -R₈₃ZR₈₃-, Z represents  N-R₈₃-A₆ or  N-A₆, R₇₉ to R₈₃ individually represent a substituted or unsubstituted alkylene group, A₂ to A₆ individually represent a hydrogen atom, -OH, -COOM or -P0₃M₂ and M is a hydrogen atom or an alkali metal atom.

Preferable illustrated compounds having the general formula (XII) and (XIII) are given below.

### Illustrated Compound

(XII - 1) Ethylenediaminetetraacetic acid
(XII - 2) Diethylenetriaminepentaacetic acid
(XII - 3) Ethylenediamine-N-(β-hydroxyethyl)-N,N',N'-triacetic acid
(XII - 4) Propylenediaminetetraacetic acid
(XII - 5) Triethylenetetraminehexaacetic acid
(XII - 6) Cyclohexanediaminetetraacetic acid
(XII - 7) 1,2-Diaminopropanetetraacetic acid
(XII - 8) 1,3-Diaminopropan-2-ol-tetraacetic acid
(XII - 9) Ethyl ether diaminetetraacetic acid
(XII - 10) Glycol ether diaminetetraacetic acid
(XII - 11) Ethylenediaminetetrapropionic acid
(XII - 12) Phenylenediaminetetraacetic acid
(XII - 13) Ethylenediaminetetraacetic acid sodium salt
(XII - 14) Ethylenediaminetetraacetic acid tetra(trimethylammonium)salt
(XII - 15) Ethylenediaminetetraacetic acid tetrasodium salt
(XII - 16) Diethylenetriaminepentaacetic acid pentasodium salt
(XII - 17) Ethylenediamine-N-(β-hydroxyethyl)-N,N',N'-triacetic acid sodium salt
(XII - 18) Propylenediaminetetraacetic acid sodium salt
(XII - 19) Ethylenediaminetetramethylene phosphonic acid
(XII - 20) Cyclohexanediaminetetraacetic acid sodium salt
(XII - 21) Diethylenetriaminepentamethylene phosphonic acid
(XII - 22) Cyclohexanediaminetetramethylene phosphonic acid
(XIII - 1) Nitrilotriacetic acid
(XIII - 2) Iminodiacetic acid
(XIII - 3) Hydroxyethyliminodiacetic acid
(XIII - 4) Nitrilotripropionic acid
(XIII - 5) Nitrilotrimethylene phosphonic acid
(XIII - 6) Iminodimethylene phosphonic acid
(XIII - 7) Hydroxyethyliminodimethylene phosphonic acid
(XIII - 8) Nitrilotriacetic acid trisodium salt

As particularly preferable compounds for the intended effects of this invention, of these aminocarboxylic acid compounds and aminophosphonic acid compounds, there may be mentioned (XII - 1), (XII - 2), (XII - 5), (XII - 8), (XII - 19), (XIII -1), (XIII - 3) and (XIII - 5).

An amount of the aminocarboxylic acid or aminophosphonic acid compounds in this invention to be added may be 10 % or less of a molar concentration of the organic acid ferric complex co-existing in a bleaching solution, preferably 0 to 5 %, more preferably 0 to 2 % for still more effective exertion of the present effects.

The ferric complex of organic acid according to this invention may be employed as a free acid (a hydroacid), an alkali metal salt such as sodium salt, potassium salt or lithium salt, an ammonium salt, a water-soluble amine salt such as triethanol amine salt, preferably potassium salt, sodium salt or ammonium salt. The ferric complexes may be employed with at least one sort thereof or in combination with 2 or more thereof. The amount to be used may be optionally selected and should be determined depending upon the silver amount of light-sensitive material to be processed, composition of a silver halide and the like; for instance, one may use not less than 0.01 mole per 1 litre of the solution employed, preferably 0.05 to 0.6 mole. And, it is preferred in a replenishing solution to employ a concentration of the solubility as condensed as possible for condensed, low replenishment.

The effect of this invention can be better exhibited and another effect to prevent the precipitation due to the silver in a bleaching solution can be also expected, when the bleaching solution contains at least one of the compounds represented respectively by General Formulae (I) to (IX) shown below, which are therefore preferably used in this invention.

In the formula, Q represents a group of atoms necessary for the formation of a nitrogen-containing heterocyclic ring (including the ring condensed with an unsaturated 5- to 6-membered ring); and R represents a hydrogen atom, an alkyl group having 1 to 6 carbon atoms, a cycloalkyl group, an aryl group, a heterocyclic ring (including the ring condensed with an unsaturated 5- to 6-membered ring) or an amino group.

In the formula, R₂ and R₃ each represent a hydrogen atom, an alkyl group having 1 to 6 carbon atoms, a hydroxyl group, a carboxyl group, an amino group, an acyl group having 1 to 3 carbon atoms, an aryl group or an alkenyl group.
A represents; or an ni -valent heterocyclic residual group (including the group condensed with an unsaturated 5- to 6- membered ring); X represents = S, = O or = NR". Here, R and R' each have the same meaning as defined for R₂ and R₃; X' has the same meaning as defined for X; Z represents a hydrogen atom, an alkali metal atom, an ammonium group, an amino group, a nitrogen-containing heterocyclic residual group, an alkyl group or M represents a divalent metallic atom; R" represents a hydrogen atom, an alkyl group having 1 to 6 carbon atoms, a cycloalkyl group, an aryl group, a heterocyclic residual group (including the group condensed with an unsaturated 5- to 6-membered ring) or an amino group; and n1 to n6 and m1 to m5 each represent an integer of 1 to 6. B represents an alkylene group having 1 to 6 carbon atoms; Y represents -N 〈 or -CH 〈 ; R₄ and R₅ each have the same meaning as defined for R₂ and R₃; provided that R₄ and R₅ each may represent -B-SZ and that R₂ and R₃, R and R', and R₄ and R₅ each may be combined to form a ring.

The compound represented by the above formula may also include an enol form compound and a salt thereof.

In the formula, R₆ and R₇ each represent a hydrogen atom, an alkyl group having 1 to 6 carbon atoms, a hydroxyl group, a carboxyl group, an amino group, an acyl group having 1 to 3 carbon atoms, an aryl group, an alkenyl group or -B₁-S-Z₁; provided that R₆ and R₇ may be combined to form a ring. Y₁ represents N- or CH-; B₁ represents an alkylene group having 1 to 6 carbon atoms; Z₁ represents a hydrogen atom, an alkali metal atom, an ammonium group, an amino group, a nitrogen-containing heterocyclic residual group or and n7 represents an integer of 1 to 6.

In the formula, R₈ and R₉ each represent or ; and R₁₀ represents an alkyl group or -(CH₂)ₙ₈SO₃^{⊖} (provided that ℓ represents 0 when R₁₀ is -(CH₂)-ₙ₈SO₃^{⊖}, or 1 when it is an alkyl group). G^{⊖} represents an anion; and n8 represent an integer of 1 to 6.

In the formula, Q₁ represents a group of atoms necessary for the formation of a nitrogen-containing heterocyclic ring (including the ring condensed with an unsaturated or saturated 5- to 6-membered ring); and R₁₁ represents a hydrogen atom, an alkali metal atom, or an alkyl group; provided that Q' have the same meaning as defined for Qi.

In the formula, D₁, D₂, D₃ and D₄ each represent a simple bond arm, an alkylene group having 1 to 8 carbon atoms or a vinylene group; and q1, q2, q3 and q4 each represent an integer of 0, 1 or 2. The ring formed together with a sulfur atom may be further condensed with a saturated or unsaturated 5- to 6- membered ring, with the exception of elementary sulfur;

In the formula, X₂ represents -COOM', -OH, -SO₃M', -CONH₂, -S0₂NH₂, -NH₂, -SH, -CN, -CO₂R₁₆, -SO₂R₁₆, -OR₁₆, -NR₁₆ R₁₇, -SR₁₆, -SO₃ R₁₆, -NHCOR₁₆, -NHS0₂ R₁₆, -OCOR₁₆ or -S0₂ R₁₆; Y₂ represents or a hydrogen atom; and m9 and n9 each represent an integer of 1 to 10. R₁₁, R₁₂, R₁₃, R₁₄, R₁₅, R₁₇ and R₁₈ each represent a hydrogen atom, a lower alkyl group, an acyl group or
R₁₆ represents a lower alkyl group;
R₁₉ represents -NR₂₀R₂₁, -OR₂₂ or -SR₂₂; R₂₀ and R₂, each represent a hydrogen atom or a lower alkyl group; and R₂₂ represents a group of atoms necessary for a ring to be formed by combination with R₁₈. R₂₀ or R₁₁ may be combined with R₁₈ to form a ring. M' represents a hydrogen atom or a cation.

In the formula, Ar represents a divalent aryl group or a divalent organic group formed by combination of an aryl group with an oxygen atom and/or alkylene group; B₂ and B₃ each represent a lower alkylene group; R₂₃, R₂₄, R₂₅ and R₂₆ each represent a hydroxyl substituted lower alkyl group; and x and y each represent 0 or 1. G' represents an anion; and z represents 0, 1 or 2.

In the formula, R₂₉ and R₃₀ each represent a hydrogen atom, an alkyl group, an aryl group or a heterocyclic group; R₃, represents a hydrogen atom or an alkyl group; R₃₂ represents a hydrogen atom or a carboxyl group.

The compounds represented respectively by General Formulae (I) to (IX) preferably used in this invention are compounds generally used as bleach accelerators, which are hereinafter referred to as the bleach accelerators of this invention.

Typical examples of the bleach accelerators of this invention may include, for example, the following, but by no means limited to these.

Besides the bleach accelerators of this invention as exemplified in the above, similarly usable compounds may also include the exemplary compounds disclosed in Japanese Patent Application No. 263568/1985 at page 51 to page 115 of the specification thereof, i.e., Compounds Nos. 1-2, I-4 to -7, I-9 to -13, 1-16 to -21, 1-23, 1-24, 1-26, 1-27, 1-30 to -36, 1-38, II-2 to -5, II-7 to -10, II-12 to -20, II-22 to -25, II-27, II-29 to -33, II-35, II-36, II-38 to -41, II-43, II-45 to -55, II-57 to -60, II-62 to -64, II-67 to -71, II-73 to -79, 11-81 to -84, II-86 to -99, II-101, II-102, 11-104 to -110, II-112 to -119, 11-121 to -124, II-126, II-128 to -144, II-146, II-148 to -155, II-157, III-4, III-6 to -8, III-10, III-11, III-13, III-15 to -18, III-20, III-22, III-23, III-25, III-27, III-29 to -32, III-35, III-36, IV-3, IV-4, V-3 to -6, V-8 to -14, V-16 to -38, V-40 to -42, V-44 to -46, V-48 to -66, V-68 to -70, V-72 to -74, V-76 to -79, V-81, V-82, V-84 to -100, V-102 to -108, V-110, V-112, V-113, V-116 to -119, V-121 to -123, V-125 to -130, V-132 to -144, V-146 to -162, V-164 to -174, V-176 to -184, VI-4, VI-7, VI-10, VI-12, VI-13, VI-16, VI-19, VI-21, VI-22, VI-25, VI-27 to -34, VI-36, VII-3, VII-6, VII-13, VII-19, VII-20, etc.

The compounds having the general formulae (I) to (IX) may be employed alone or in combination with two or more thereof and an amount of the bleaching accelerator to be added to a bleaching solution is usually in the range of 0.01 to 100 g per one litre of the processing solution to give favourable results. In General, however, when an added amount is too small, a bleaching acceleration effect is less, while when an added amount is too large over the required level, precipitates may be formed to stain the light-sensitive silver halide color photographic material to be processed. Accordingly, 0.05 to 50 g per one litre of the processing solution may be preferable, more preferably 0.05 to 15 g per one litre of the processing solution.

The present compounds having the above general formulae (I) to (IX) when added to a bleaching solution may be added and dissolved as such, but generally added after previously dissolved in water, an alkali, an organic acid, etc. and, where necessary, they may be added as dissolved in an organic solvent such as methanol, ethanol or acetone to produce no influence upon their bleaching effect and the above-depicted effects.

A processing time for bleaching of a light-sensitive silver halide color photographic material with the present bleaching solution is preferably short in order to exert the present effects more effectively. Preferable bleaching time is 6 minutes or shorter, more preferably it is 4 minutes or shorter.

The present bleaching solution may be employed at a pH value of 0.2 to 9.5, preferably 2.0 to 8.0, more preferably 4.0 to 7.0. Processing temperature may be 80 _{°} C or lower, desirably 55 _{°} C or lower for preventing evaporation and other.

Generally, the present bleaching solution may contain a halide such as ammonium bromide and the like.

Also, the present bleaching solution may contain a pH buffering agent alone or in combination with two or more thereof, said buffering agent comprising various salts such as boric acid, borax, sodium hydroxide, potassium hydroxide, sodium carbonate, potassium carbonate, sodium bicarbonate, potassium bicarbonate, acetic acid, sodium acetate, ammonium hydroxide and the like. Further, a variety of brightening agents, defoaming agents, surfactants, mildewproofing agents and the like may be incorporated into the bleaching solution.

The aromatic primary amine color developing agent which may be preferably employed in the present color developing solution may include various agents widely employed in a variety of color photographic processings. Such developing agents may involve aminophenol- and p-phenylenediamine-type derivatives.

These compounds may be generally employed in the form of a salt, e.g., hydrochloride or sulfate rather stable than the free form. They may be usually employed at a concentration of about 0.1 g to about 50 g per one litre of a color developer, more preferably about 1 g to about 1.5 g per one litre of the developer.

As the aminophenol-type developer, there may be mentioned, for example, o-aminophenol, p-aminophenol, 5-amino-2-oxytoluene, 2-amino-3-oxytoluene, 2-oxy-3-amino-1,4-dimethylbenzene and the like.

Particularly useful aromatic primary amine color developing agents in view of the intended objects of this invention are the aromatic primary amine color developing agent containing an amino group having at least one water-soluble group, and the compounds having the following general formula [X] are especially preferred.

In this formula, R represents a hydrogen atom, a halogen atom, or an alkyl group, said alkyl group having a straight or branched chain of 1 to 5 carbon atoms and optionally a substituent. R₁₄ and R₁₅ individually represent a hydrogen atom, an alkyl group or an aryl group, said alkyl or aryl group being optionally substituted. In the case of alkyl groups, there is mentioned preferably an alkyl group substituted with an aryl group. At least one of R₁₄ and R₁₅ is an alkyl group substituted with a water-soluble group such as a hydroxy group, a carboxy group, a sulfonic acid group, an amino group, a sulfonamido group and the like or said alkyl group being optionally further substituted. R₁₆ represents a hydrogen atom or an alkyl group having a straight or branched chain of 1 to 5 carbon atoms and p and q each is an integer of 1 to 5.

Examples of the compounds having the above general formula [X] are given below, but the present compounds are not limited thereto.

### [Exemplary Compound]

The p-phenylenediamine derivatives having the above general formula (X) may be employed as salts with an organic or inorganic acid and, for example, one may employ hydrochloride, sulfate, phosphate, p-toluenesulfonate, sulfite, oxalate, benzenedisulfonate and the like.

The color developing solution which may be employed in this invention may optionally further contain various components commonly applied, for example, an alkali agent such as sodium hydroxide, sodium carbonate and the like; an alkali metal sulfite; an alkali metal hydrosulfite; an alkali metal thiocyanate, an alkali metal halide; benzyl alcohol; a softening agent; a thickner; a developing accelerator; and the like.

Next, cyan coupler according to this invention will be described below.

The cyan coupler of this invention can be represented by Formula (C) shown below. wherein R₂, represents an alkyl group, an alkenyl group, a cycloalkyl group, an aryl group or a heterocyclic group.

Herein, R₂, represents an alkyl group, preferably an alkyl group having 1 to 20 carbon atoms (for example, each group of methyl, ethyl, t-butyl, dodecyl, etc.), an alkenyl group, preferably an alkenyl group having 2 to 20 carbon atoms (such as an allyl group and a heptadecenyl group), a cycloalkyl group, preferably 5- to 7-membered one (for example, cyclohexyl, etc.), an aryl group (for example, a phenyl group, a tolyl group, a naphthyl group, etc.), a heterocyclic group, preferably a group of 5- or 6-membered ring containing 1 to 4 nitrogen atom(s), oxygen atom(s) or sulfur atom(s) (for example, a furyl group, a thienyl group, a benzothiazolyl group, etc.).

Into R₂, a desirable substituent may be introduced, for example, an alkyl group having 1 to 10 carbon atoms (for example, methyl, i-propyl, i-butyl, t-butyl, t-octyl, etc.), an aryl group (for example, phenyl, naphthyl, etc.), a halogen atom (such as fluorine, chlorine and bromine), cyano, nitro, a sulfonamide group (for example, methanesulfonamide, butanesulfonamide, p-toluenesulfonamide, etc.), a sulfamoyl group (such as methylsulfamoyl and phenylsulfamoyl) a sulfonyl group (for example, methanesulfonyl, p-toluenesulfonyl, etc.), a fluorosulfonyl group, a carbamoyl group (for example, dimethyl carbamoyl group, phenyl carbamoyl group, etc.), an oxycarbonyl group (for example, ethoxycarbonyl, phenoxycarbonyl, etc.), an acyl group (for example, acetyl, benzoyl, etc.) a hetero ring (for example, a pyridyl group, a pyrazolyl, etc.), an alkoxy group, an aryloxy group, an acyloxy group, etc.

R₂, represents a ballast group necessary for imparting diffusion resistance, to the cyan coupler represented by Formula (C) and a cyan dye to be formed from said cyan coupler. Preferably, it is an alkyl group having 4 to 30 carbon atoms, an aryl group, an alkenyl group, a cycloalkyl group or a heterocyclic group. For example, it may include a straight chain or branched alkyl group (for example, t-butyl, n-octyl, t-octyl, n-dodecyl, etc.), a 5- or 6-membered heterocyclic group, etc.

In Formula (C), R₂₄ represents a substituted or unsubstituted aryl group (particularly preferably a phenyl group). The substituent in the case when said aryl group have a substituent may include at least one of substituents selected from S0₂ R₂₅, a halogen atom (such as fluorine, chlorine, bromine, etc.), -CF₃, -N0₂, -CN, -COR₂₅, -COOR₂₅, -S0₂₅ OR₂₅, -OR₂s, -OCOR₂₅, and

Herein, R₂₅ represents an alkyl group, preferably an alkyl group having 1 to 20 carbon atoms (for example, each group of methyl, ethyl, t-butyl and dodecyl), an alkenyl group, preferably an alkenyl group having 2 to 20 carbon atoms (such as an allyl group and heptadecenyl group), a cycloalkyl group, preferably 5- to 7-membered one (for example, cyclohexyl, etc.) an aryl group (for example, a phenyl group, a tolyl group, a naphtyl group, etc.); and R₂₆ represents a hydrogen atom or the group represented by R₂₅.

A preferable compound of the cyan coupler of this invention, represented by Formula (C), is a compound such that R₂₄ is a substituted or unsubstituted phenyl group, and the substituent for the phenyl group is cyano, nitro, -S0₂ R₂₇ (R₂₇ is an alkyl group), a halogen atom or trifluoromethyl.

Preferred examples of the ballast group represented by R₂₁ include a group represented by Formula (C - 1)) shown below.

In the formula, J represents an oxygen atom or a sulfonyl group; K represents an integer of 0 to 4; R represents 0 or 1; and R₂₉ which is present in two or more numbers when K comprises two or more, may be the same or different; R₂₈ represents a straight or branched alkylene group having 1 to 20 carbon atoms and substituted with an aryl group, etc.; and R₂₉ represents a monovalent group, preferably, a hydrogen atom, a halogen atom (for example, chlorine, bromine, etc.), an alkyl group, preferably a straight or branched alkyl group having 1 to 20 carbon atoms (for example, each group of methyl, t-butyl, t-pentyl, t-octyl, dodecyl, pentadecyl, benzyl, phenetyl, etc.), an aryl group (for example, a phenyl group), a heterocyclic group (for example, a nitrogen-containing heterocyclic group), an alkoxy group, preferably a straight chain or branched alkoxy group having 1 to 20 carbon atoms (for example, each group of methoxy, ethoxy, t-butyloxy, octyloxy, decyloxy, dedecyloxy group, etc.), an aryloxy group (for example, a phenoxy group), a hydroxyl group, an acyloxy group, preferably an alkylcarbonyloxy group, an arylcarbonyloxy group (for example, an acetoxy group and benzoyloxy group), carboxy, alkyloxycarbonyl group, preferably a straight or branched alkylcarbonyl group having 1 to 20 carbon atoms, more preferably a phenoxycarbonyl group, an alkylthio group, preferably an acyl group having 1 to 20 carbon atoms, more preferably a straight or branched alkylcarbonyl group having 1 to 20 carbon atoms, an acylamino group, preferably a straight chain or branched alkylcarbamide group having 1 to 20 carbon atoms, a benzenecarbamide group, a sulfonamide group, preferably a straight chain or branched alkylsulfonamide group having 1 to 20 carbon atoms or a benzenesulfonamide group, a carbamoyl group, preferably a straight chain or branched alkylaminocarbonyl group having 1 to 20 carbon atoms or a phenylaminocarbonyl group, sulfamoyl group, preferably a straight chain or branched alkylaminosulfonyl group having 1 to 20 carbon atoms or a phenylaminosulfonyl group, etc.

In Formula (C) Z represents a hydrogen atom or a group eliminatable through a coupling reaction with an oxidized product of the N-hydroxyalkyl substituted-p-phenylenediamine derivative color developing agent. For example, it may include a halogen atom (for example, chlorine, bromine, fluorine, etc.), a substituted or unsubstituted alkoxy group, an aryloxy group, a heterocyclic oxy group, an acyloxy group, a carbamoyloxyl group, a sulfonyloxy group, an alkylthio group, an arylthio group, a heterocyclic thio group, a sulfonamide group, etc., and more specific examples may include those described in U.S. Patent No. 3,741,563, Japanese Unexamined Patent Publication No. 37425/1972, Japanese Patent Publication No. 36894/1973, Japanese Unexamined Patent Publications No. 10135/1975, No. 117422/1975, No. 130441/1975, No. 108841/1976, No. 120343/1975, No. 18315/1977, No. 105226/1978, No. 14736/1979, No. 48237/1979, No. 32071/1980, No. 65957/1980, No. 1938/1981, No. 12643/1981, No. 27147/1981, No. 146050/1984, No. 166956/1984, No. 24547/1985, No. 35731/1985 and No. 37557/1985; etc.

Specific exemplary compounds for the cyan coupler represented by Formula (C) of this invention are shown below, but by no means limited to these.

These cyan couplers of this invention can be synthesized by known methods, for example, synthesis methods as described in U.S. Patents No. 3,222,176, No. 3,446,622 and No. 3,996,253; British Patent No. 1,011,940; Japanese Unexamined Patent Publications No. 21139/1972, No. 65134/1981, No. 204543/1982 and No. 204544/1982; Japanese Unexamined Patent Publications No. 33250/1983, No. 33248/1983, No. 33249/1983, No. 33251/1983, No. 33252/1983 and No. 31334/1983; Japanese Unexamined Patent Publications No. 24547/1985, No. 35731/1985 and No. 37557/1985; etc.

The cyan couplers represented by Formula (C) of this invention may be used alone or in combination of two or more kinds. When the cyan couplers of this invention is contained in a silver halide emulsion layer, an amount thereof is usually about 0.005 2 mole, preferably 0.01 to 1 mole per 1 mole of silver halide contained in the silver halide emulsion layer.

The photographic material in carrying out the method of the present invention, is one which contains, in at least one layer of the silver halide emulsion layer thereof, a magenta coupler represented by the formula (M).

When the substituent (e.g. R, R₁ to Rs) on the hetero- cyclic ring in the formula (M) and the formulae (M - I) to (M - VI) as hereinafter described has a moiety of the formula: (wherein R", X and Z" have the same meanings as R, X and Z in the formula (M)), the so-called bis-form type coupler is formed, which is of course included in the present invention. The ring formed by Z, Z', Z" and Z₁ as hereinafter described may also be fused with another ring (e.g. a 5- to 7-membered cycloalkene). For example, R₅ and R₆ in the formula (M - IV), R₇ and R₈ in the formula (M - V) may be bonded to each other to form a ring (e.g. a 5- to 7-membered rings).

The compounds represented by the formula (M) can be also represented specifically by the following formulae (M - I) through (M - VI).

In the above formulae (M - I) to (M - VI)), R₁ to R₈ and X have the same meanings as the above R and X.

Of the compounds represented by the formula (M), those represented by the following formula (M - VII) are preferred. wherein Ri, X and Z₁ have the same meanings as R, X and Z in the formula (M.

Of the magenta couplers represented by the formulae (M - I) to (M - VI), the magenta coupler represented by the formula (M - I)) is particularly preferred.

To describe about the substituents on the heterocyclic ring in the formulae (M) and (M - I) to (M - VII), R in the formula (M) and R₁ in the formulae (M - I) to (M - VII) should preferably satisfy the following condition 1, more preferably satisfy the following conditions 1 and 2, and particularly preferably satisfy the following conditions 1, 2 and 3:
Condition 1: a root atom directly bonded to the heterocyclic ring is a carbon atom,
Condition 2: only one of hydrogen atom is bonded to said carbon atom or no hydrogen atom is bonded to it, and
Condition 3: the bondings between the root atom and adjacent atoms are all single bonds.

Of the substituents R and R₁ on the above heterocyclic ring, most preferred are those represented by the formula (M - VIII) shown below:

In the above formula, each of R₉, R₁₀ and R₁₁ represents a hydrogen atom, a halogen atom, an alkyl group, a cycloalkyl group, an alkenyl group, a cycloalkenyl group, an alkynyl group, an aryl group, a heterocyclic group, an acyl group, a sulfonyl group, a sulfinyl group, a phosphonyl group, a carbamoyl group, a sulfamoyl group, a cyano group, a spiro compound residual group, a bridged hydrocarbon compound residual group, an alkoxy group, an aryloxy group, a heterocyclicoxy group, a siloxy group, an acyloxy group, a carbamoyloxy group, an amino group, an acylamino group, a sulfonamide group, an imide group, an ureido group, a sulfamoylamino group, an alkoxycarbonylamino group, an aryloxycarbonylamino group, an alkoxycarbonyl group, an aryloxycarbonyl group, an alkylthio group, an arylthio group or a heterocyclicthio group. At least two of R₉, R₁₀ and R₁₁ are not hydrogen atoms at the same time.

Also, at least two of said R₉, R₁₀ and R₁₁, for example, R₉ and R₁₀ may be bonded together to form a saturated or unsaturated ring (e.g. cycloalkane ring, cycloalkene ring or heterocyclic ring), and further to form a bridged hydrocarbon compound residual group by bonding R₁₁ to said ring.

The groups represented by R₉ to R₁₁ may have substituents, and examples of the groups represented by R₉ to R₁₁ and the substituents which may be possessed by said groups may include examples of the substituents which may be possessed by the R in the above formula (M), and substituents which may be possessed by said substituents.

Also, examples of the ring formed by bonding between R₉ and Rio, the bridged hydrocarbon compound residual group formed by R₉ to R₁₁ and the substituents which may be possesed thereby may include examples of cycloalkyl, cycloalkenyl and heterocyclic groups as mentioned for substituents on the R in the aforesaid formula (M) and substituents thereof.

Of the groups of the formula (M - VIII), preferred are:
(i) the case where two of R₉ to R₁₁ are alkyl groups; and
(ii) the case where one of R₉ to R₁₁, for example, R₁₁ is a hydrogen atom and two of the other R₉ and R₁₀ are bonded together with the root carbon atom to form a cycloalkyl group.

Further, preferred in (i) is the case where two of R₉ to R₁₁ are alkyl groups and the other one is a hydrogen atom or an alkyl group.

Here, said alkyl and said cycloalkyl may further have substituents, and examples of said alkyl, said cycloalkyl and subsituents thereof may include those of alkyl, cycloalkyl and substituents thereof as mentioned for the substituents on the R in the formula (M) and the substituents thereof.

The magenta coupler represented by formula (M) may include the specific compound enumerated below.

Magenta couplers for photography which may be combined with the magenta coupler of this invention may include compounds of pyrazolone type, pyrazolinobenzimidazole type, and indazolone type, etc. The pyrazolone type magenta couplers may include the compounds disclosed in U.S Patents No. 2,600,788, No. 3,062,653, No. 3,127,269, No. 3,311,476, No. 3,419,391, No. 3,519,429, No. 3,558,318, No. 3,684,514 and No. 3,888,680, Japanese Unexamined Patent Publications No. 29639/1974, No. 111631/1974, No. 129538/1974 and No. 13041/1975, Japanese Patent Publications No. 47167/1978, No. 10491/1979 and No. 30615/1980. As nondiffusion colored magenta couplers, there may be generally used the compounds arylazo-substituted at the coupling position of a colorless magenta coupler, which may include, for example, the compounds disclosed in U.S. Patents No. 2,801,171, No. 2,983,608, No. 3,005,712 and No. 3,684,514, British Patent No. 937,621, Japanese Unexamined Patent Publications No. 123625/1974 and No. 31448/1974.

The colored magenta couplers of the type such that a dye may flow out into a processing solution by the reaction with an oxidized product of a developing agent, as disclosed in U.S. Patent No. 3,419,391, can be also used.

In the light-sensitive silver halide photographic material employed for the processing method of this invention, there may preferably be contained a pyrazoloasol type magenta coupler having at least one aromatic sulfonyl group represented by Formula (A) in the molecular structure.

The pyrazoloasol type magenta coupler having at least one aromatic sulfonyl group represented by Formula (A) in the molecular structure employed for this invention may preferably be a magenta coupler represented by the following formula (M). wherein Z represents non-metal atoms necessary for formation of a nitrogen-containing heterocyclic ring, the ring formed by said Z may have a substituent; X represents a hydrogen atom or a group eliminatable through the reaction with an oxidzed product of a color developing agent; R represents a hydrogen atom or a substituent, provided that R is a substituent and/or the ring formed by Z has a substituent, and at least one of said substituent has the group represented by Formula (A).

The aromatic sulfonyl group represented by Formula (A) will be described below in detail Formula (A):

In the formula, R represents an aliphatic group, an aryl group or a heterocyclic group; m represents an integer of 1 or 2; and R may be the same or different when m is 2. R₂ represents an aliphatic group, an aryl group, a heterocyclic group or (wherein R3 and R4 each represent a hydrogen atom, aliphatic group or an aryl group).

In Formula (A), to describe R and R₂ in further detail, the aliphatic group is preferably an aliphatic group having 1 to 36 carbon atoms, including a straight chain or branched alkyl group, an alkenyl group, an aralkyl group, a cycloalkyl group, an alkynyl group and a cycloalkenyl group, and these aliphatic groups may include those having a substituent, which substituent may include the groups other than hydrogen mentioned for the above R. The aryl group may include, for example, a phenyl group, a naphthalene group, etc., and may include those having a substituent, which substituent may include the groups other than hydrogen mentioned for the above R. The heterocyclic group may preferably include a 5- to 7-membered ring containing at least one selected from 1 to 4 nitrogen atom(s), oxygen atom(s) and sulfur atom(s) (for example, a furyl group, a thienyl group, a pyrimidinyl group, an imidazolyl group, a pyrazolyl group, a benzothiazolyl group, a piperidino group, a morpholino group, a benzimidazolyl group, triazolyl group, a triazine group, etc.). These may include those having a substituent, which substituent may include the groups other than hydrogen mentioned for the above R. The group of may preferably include a di-substituted amino group substituted with an aliphatic group or aryl group.

Of the aromatic sulfonyl group represented by Formula (A), preferable is the compound represented by the following formula:

In the formula, R₁₂ and R₁₃ each represent a group having the same meaning as defined for R and R₂ in Formula (A).

More preferable is the compound wherein R₁₂ is an alkyl group. Particularly preferable is the compound wherein R₁₃ is an aryl group substituted with an alkoxy group.

Typical examples of the magenta coupler used in this invention are shown below, but by no means limited to these.

The pyrazoloazole type magenta coupler having at least one aromatic sulfonyl group represented by Formula (A) in the molecular structure of this invention can be synthesized by making reference to Journal of the Chemical Society, Perkin I (1977), 2047-2052, U.S. Patent No. 3,725,067, Japanese Unexamined Patent Publications No. 99437/1984, No. 42045/1983, No. 162548/1984, No. 171956/1984, No. 33552/1985, No. 43659/1985, No. 172982/1985 and No. 190779/1985, etc.

The pyrazoloazole type magenta coupler of this invention can be used generally in the range of 1 x 10-³ mole to 1.5 moles, preferably 1 x 10-² mole to 1 mole, per mole of silver halide.

The pyrazoloazole type magenta coupler of this invention can be used in combination with other type of magenta couplers.

The pyrazoloazole type magenta coupler of this invention may be added to a desired hydrophilic colloid layer after dissolving it in an organic solvent having a high boiling point of about 150°C or more optionally together with a low boiling solvent and/or a water soluble organic solvent and effecting emulsification dispersion of the solution in a hydrophilic binder such as an aqueous gelatin solution with use of a surface active agent. There may be inserted a step of removing the dispersing solution, or at the same time of the dispersion, the low boiling organic solvent.

As another preferred embodiment of this invention, it has been found out that the object of this invention can be much more effectively accomplished by incorporating into the light-sensitive silver halide photographic material at least one of the compounds having the following general formula (XI).

In this formula, Z₁₁ and Z₂₁ individually represent atom groups required for forming a benzene or naphthalene ring condensed to an oxazole ring. R41 and R₄₂ indivually represent an alkyl group, an alkenyl group, or an aryl group, R₄₃ represents a hydrogen atom or an alkyl group having 1 to 3 carbon atoms, X₁- represents an anion, and n is 1 or 0.

The definitions of the general formula [XI] are illustrated in detail.

In the formula, Z₁₁ and Z₂, each represent a group of atoms necessary for the formation of a benzene ring or naphthalene ring condensed with an oxazole ring. The heterocyclic ring to be formed may be substituted with a substituent of various types, and these substituents may preferably include a halogen atom, an aryl group, an alkenyl group, an alkyl group and an alkoxy group. More preferable substituents are a halogen atom, a phenyl group and a methoxy group, and the most preferable substituent is a phenyl group.

Preferable embodiment is that Z₁₁ and Z₂, both represent benzene rings condensed with oxazole rings, respectively, and at least one benzene ring of these benzene rings is substituted with a phenyl group at the 5-position thereof and with a halogen atom at the 5-position of the other benzene ring. R41 and R₄₂ each represent an alkyl group, an alkenyl group or an aryl group, and preferably represent an alkyl group. More preferably, R₄₁ and R₄₂ each represent an alkyl group substituted with a carboxyl group or sulfo group, and most preferably, a sulfoalkyl group having 1 to 4 carbon atoms. Still most preferably, they each are a sulfoethyl group. R₄₃ represents a hydrogen atom or an alkyl group having 1 to 3 carbon atoms, and preferably represent a hydrogen atom or an ethyl group. X₁ - represents an anion; and n represents 0 or 1.

The sensitizing dye represented by General Formula (XI), used in this invention, can also be used in combination with other sensitizing dyes as a so-called supersensitizing combination. In such an occasion, the respective sensitizing dyes may be dissolved in solvents of the same or different type, and these solutions may be mixed prior to the addition to an emulsion or separately added to the emulsion. When they are separately added, the order and the time interval may be arbitrarily determined depending on the purpose.

Specific examples of the sensitizing dye represented by General Formula (XI) are shown below, but the sensitizing dyes used in this invention are by no means limited to these compounds.

The sensitizing dye having the above general formula (XI) may be added to an emulsion at any point during the preparation of the emulsion and preferably during or after chemical ripening. An amount of the dye to be added may be preferably 2 x 10-⁶ mole to 1 x 10-³ mole per 1 mole of a silver halide, more preferably 5 x 10-⁶ mole to 5 x 10-⁴ mole per 1 mole of the halide.

As the silver halide emulsion which may be employed in this invention, there may be any emulsion using any silver halide such as silver chloride, silver bromide, silver iodide, silver chlorobromide, silver chloroiodide, silver iodobromide or silver chloroiodobromide. As the protective colloid for these silver halides, one may use natural products such as gelatin and the like or various synthetic products. The silver halide emulsion may also contain conventional photographic additives such as a stabilizer, a sensitizer, a hardening agent, a sensitizing dye, a surfactant and others.

The processing method according to this invention may be applicable to light-sensitive silver halide color photographic materials such as a color paper, a negative color film, a positive color film, a color reversal film for slide, a color reversal film for motion picture, a color reversal film for TV or a color reversal paper, . In particular, the present method is most suited to processing of a high-sensitive light-sensitive color photographic material containing the silver iodobromide or chloroiodobromide containing 0.1 mole % or more of silver iodide and having a total coated silver amount of not less than 20 mg/dm^{2.}

### Comparative Example 1

An antihalation coating layer and a gelatin layer were coated over a triacetate film base and there were then coated thereover, in turn, a red-sensitive silver halide emulsion layer, a green-sensitive silver halide emulsion layer, a filter layer containing yellow colloidal silver, a blue-sensitive silver halide emulsion layer and a protective layer so that a total silver amount may become 60 mg per 100 cm^{2.} Said emulsion layers contained individually a mole % of silver iodide of about 4.5 % of silver iodobromide, while the following yellow coupler (Y - 1) was applied for the blue-sensitive silver halide emulsion layer, the following magenta coupler (M' - 1) for the green-sensitive silver halide emulsion layer and the following cyan coupler (C' - 1) for the red-sensitive silver halide emulsion layer, respectively.

Further, there may be optionally applied such conventional additives as a high-boiling solvent, a sensitizing dye, a hardening agent, a spreader and the like. The negative color films thus produced were exposed, respectively, according to conventional procedures and then subjected to running processing according to the under-mentioned development processing steps.

The color developing solution, bleaching solution, fixing solution and stabilizing solution as prescribed below were employed.

### [Color developing solution]

Water was added to make up a 1 litre volume and a pH value was adjusted to 10.06 with potassium hydroxide or 20 % sulfuric acid.

### [Bleaching solution and bleaching replenisher]

Water was added to make up a 1 litre volume and a pH value was adjusted to 6.0 with acetic acid with aqueous ammonia.

### [Fixing solution and fixing replenisher]

Water was added to make up a 1 litre volume and a pH value was adjusted to 7.0 with acetic acid and aqueous ammonia.

### [Stabilizing solution and stabilizing replenisher]

Water was added to make up a 1 litre volume.

### [Color development replenisher]

Water was added to make up a 1 litre volume and a pH value was adjusted to 10.12 with potassium hydroxide or 20 % sulfuric acid.

The bleaching replenisher, fixing replenisher and stabilizing replenisher were used with the same compositions as in the respective tank solutions. Also, concentrations of the ethylenediaminetetraacetic acid as one example of the organic acid involved in the bleaching solution varied as indicated in the following Table 1.

The color development replenisher was supplied to the color developing solution at 1.5 R per 1 m² of the negative color film and the fixing replenisher to the fixing bath at 1 R per 1 m² of the negative color film. Also, the stabilizing replenisher was supplied at 1 R per 1 m² of the negative color film and washing water was flown at 15 ℓ per 1 m² of the film. The bleaching replenisher was supplied at a replenished volume as indicated in the following Table 1.

Continuous running processing was applied to 50 m² of a negative color film, during which a pH value of the bleaching solution was properly adjusted to pH 6.0. The processed sample after running processing was measured for a density of the cyan dye in the maximum density band by means of "Sakura" photoelectric densitometer PDA-65 (available from Konishiroku Photo Industry Co., Ltd.). Also, recoloring property was determined from a difference in the cyan dye density between the sample and the sample retreated with red prussiate. A residual silver amount in the maximum density band was measured according to a fluorescent X-ray method. The above results are summarized in Table 1.

As apparent from the results in the above Table 1, recoloring property of cyan dye and desilvering property are greatly deteriorated when a replenished amount of the bleaching solution is reduced to not more than 300 mî per 1 m² of the negative color film; however, it is shown that the bleaching solution having a concentration of ethylenediaminetetraacetic acid, one example of the organic acids involved in the bleaching solution, within the perview of this invention does show an extremely slight deterioration in both recoloring and desilvering properties, even though a replenished amount of the bleaching solution is greatly lowered.

### Example 2

An antihalation layer and a gelatin layer were coated over a triacetate film base and there were then coated thereover, in turn, a red-sensitive silver halide emulsion layer, a green-sensitive silver halide emulsion layer, a filter layer containing yellow colloidal silver, a blue-sensitive silver halide emulsion layer and a protective layer so that a total silver amount may beocme 72 mg per 100 cm^{2.} Said emulsion layers contained individually a mole % of silver iodide of about 4.3 % of silver iodobromide, while the yellow coupler (Y - 1) as used in Comparative Example 1 was used for the blue-sensitive silver halide emulsion layer, the said Exemplary magenta coupler (M - 5) for the green-sensitive silver halide emulsion layer and the cyan coupler (C'-1) as used in Comparative Example 1 for the red-sensitive silver halide emulsion layer.

Further, there may be optionally applied such convenient additives as a high-boiling solvent, a sensitizing dye, a hardening agent, a spreader and the like. The negative color films thus produced were exposed, respectively, according to conventional procedures and then subjected to running processing according to the same development processing steps as in Comparative Example 1 except that a concentration of ethylenediaminetetraacetic acid, one example of the organic acids involved in the bleaching solution, was changed as shown in the following Table 3.

In the steps, continuous running processing was done for 40 m² of a negative color film, during which a pH value was properly adjusted to pH 6.0. After completion of the running processing, the processed sample was allowed to stand at 38 _{°} C for 3 days and then measured for a density of the cyan dye in the maximum density band by means of "Sakura" photoelectric densitometer PDA-65 (available from Konishiroku Photo Industry Co., Ltd.). Recoloring property was also determined from a difference in the cyan dye density between the sample and the sample retreated with a red prussiate solution, while a residual silver amount in the maximum density band was measured. The results are summarized in Table 3.

As apparent from the results of Table 3, where a replenished amount of the bleaching solution is reduced to not more than 300 ml per 1 m² of the negative color film, recoloring and desilvering properties of the cyan dye was greatly deteriorated; however, it is seen that both recoloring and desilvering properties can be greatly improved with the bleaching solution wherein a concentration of ethylenediaminetetraacetic acid falls within the range of this invention.

### Example 3

Comparative samples were prepared by replacing the magenta coupler (M - 5) employed for the film sample of Example 2 with the comparative magenta coupler (M' - 1) as used in Example 2 and the comparative magenta coupler (M' - 2) as shown below repspectively. Also, the film samples of this invention were similarly prepared by using the Exemplary magenta couplers (M - 18), (M - 44), (M - 59), (M - 7), (M - 22), (M - 104), (M - 127) and (M - 1), respectively. After storing for 3 days, processing was carried out by using the bleaching solution of Example 2, test No. 44. Magenta stain in unexposed portion was measured. As a result, the samples using the present magenta couplers showed in every case less magenta stain by 0.04 to 0.06, as compared with the magenta coupler out of the present invention.

### Example 4

Following the same procedures as in Examples 2, tests were carried out, except that the Exemplary Compounds (II - 28), (II - 144), (III - 34), (III - 2), (III - 38) (V - 71), (V - 75) and (VIII - 1) were applied to the bleaching solutions used in Example 2, test Nos. 41 to 45, respectively, and the bleaching processing time was 2 minutes. As a result, though the bleaching processing time was shortened, a residual silver amount in every case was reduced by about 15 to 20 %.

### Example 5

Following the same procedures as in Example 2, there were prepared film samples, except that the Exemplary Compound (XI - 1) or (X - 4) was applied to the green-sensitive silver halide emulsion layer of the film sample prepared by Example 1, and then the same tests as in Example 2 were effected. As a result, a residual silver amount was reduced by 5 to 10 % when the present bleaching solution was applied.

### Example 6

An antihalation coating layer and a gelatin layer were coated over a triacetate film base and there were then coated thereover, in turn, a red-sensitive silver halide emulsion layer, a green-sensitive silver halide emulsion layer, a filter layer containing yellow colloidal silver, a blue-sensitive silver halide emulsion layer and a protective layer so that a total silver amount may become 65 mg per 100 cm^{2.} Said emulsion layers contained individually a mole % of silver iodide of about 4.2 % of silver iodobromide, while the above-mentioned yellow coupler (Y - 1) was applied for the blue-sensitive silver halide emulsion layer, the above-mentioned Exemplary magenta coupler (M - 203) for the green-sensitive silver halide emulsion layer and the above-mentioned cyan coupler (C' - 1) for the red-sensitive silver halide emulsion layer, respectively. As a supersensitizing agent, the following (Z - 1) was employed.

Further, there may be optionally applied such conventional additives as a high-boiling solvent, a hardening agent, a spreader and the like. The negative color films thus produced were exposed, respectively, according to conventional procedures and then subjected to running processing according to the under-mentioned development processing steps.

The color developing solution, bleaching solution, fixing solution and stabilizing solution as prescribed below were employed.

### [Color developing solution]

Water was added to make up a 1 litre volume and a pH value was adjusted to 10.00 with potassium hydroxide or 20 % sulfuric acid.

### [Bleaching solution and bleaching replenisher]

Water was added to make up a 1 litre volume and a pH value was adjusted to 5.9 with acetic acid with aqueous ammonia.

### [Fixing solution and fixing replenisher]

Water was added to make up a 1 litre volume and a pH value was adjusted to 7.0 with acetic acid and aqueous ammonia.

### [Stabilizing solution and stabilizing replenisher]

Water was added to make up a 1 litre volume.

### [Color development replenisher]

Water was added to make up a 1 litre volume and a pH value was adjusted to 10.12 with potassium hydroxide or 20 % sulfuric acid.

The bleaching replenisher, fixing replenisher and stabilizing replenisher were used with the same compositions as in the respective tank solutions. Also, concentrations of the ethylenediaminetetraacetic acid as one example of the organic acid involved in the bleaching solution varied as indicated in the following Table 4.

The color development replenisher was supplied to the color developing solution at 1.5 R per 1 m² of the negative color film and the fixing replenisher to the fixing bath at 1 R per 1 m² of the negative color film. Also, the stabilizing replenisher was supplied at 1 R per 1 m² of the negative color film and washing water was flown at 15 ℓ per 1 m² of the film. The bleaching replenisher was supplied at a replenished volume as indicated in the following Table 4.

Continuous running processing was applied to 40 m² of a negative color film, during which a pH value of the bleaching solution was properly adjusted to pH 6.0. The processed sample after running processing was measured for a density of the cyan dye in the maximum density band by means of "Sakura" photoelectric densitometer PDA-65 (available from Konishiroku Photo Industry Co., Ltd.). Also, recoloring property was determined from a difference in the cyan dye density between the sample and the sample retreated with red prussiate. A residual silver amount in the maximum density band was measured according to a fluorescent X-ray method. The above results are summarized in Table 4.

As apparent from the results in the above Table 4, recoloring property of cyan dye and desilvering property are greatly deteriorated when a replenished amount of the bleaching solution is reduced to not more than 300 mî per 1 m² of the negative color film; however, it is shown that the bleaching solution having a concentration of ethylene-diaminetetraacetic acid, one example of the organic acids involved in the bleaching solution, within the perview of this invention does show an extremely slight deterioration in both recoloring and desilvering properties, even though a replenished amount of the bleaching solution is greatly lowered.

### Example 7

Comparative samples were prepared by replacing the magenta coupler (M - 203) employed for the film sample of Example 6 with the comparative magenta coupler (M' - 1) as used in Example 1 and the comparative magenta coupler (M' - 2) as used in Example 3. Also, the film samples of this invention were similarly prepared by using the Exemplary magenta couplers (M - 200), (M - 216), (M - 220), (M - 228), (M - 233), (M - 235), (M - 239), (M - 205), (M - 209) and (M - 245) respectively. After storing for 3 days, processing was carried out by using the bleaching solution of Example 6, test No. 69. Cyan dye density and residual silver amount were measured. Also, magenta stain in unexposed portion was measured.

Results are also shown in Table 5.

As a result, the samples using the present magenta couplers showed in every case less magenta stain by 0.04 to 0.06, as compared with the magenta coupler out of the present invention.

There are also found that both the recoloring properties of cyan dye and the residual silver amount were good.

### Example 8

Following the same procedures as in Example 6, tests were carried out, except that the Exemplary Compounds (I - 2), (I - 9), (II - 28), (II - 26), (II - 158) (III - 33), (III - 34), (III - 37), (IV - 1 (V - 71), (V - 185), (V - 186), (VI - 8), (VI - 9), (VII - 3), (VIII - 1), (VIII - 4) and (IX - 1) were applied to the bleaching solutions used in Example 6, test No. 69 in the amount described in Table 6, respectively, and the bleaching processing time was 3 minutes.

As a result, though the bleaching processing time was shortened, a residual silver amount in every case was reduced.

### Example 9

Following the same procedures as in Example 6, there were prepared film samples, except that the Exemplary Compound (XI - 1) (XI - 4), (XI - 6) and (XI - 11) were applied to the green-sensitive silver halide emulsion layer of the film sample prepared by Example 6, and then the same tests as in Example 2 were effected. Results are shown in Table 7.

From the result of Table 7, there are found that, in the case where the breaching solution and the sensitizing dye of the present invention were employed in combination, residual silver amount was further reduced by about one third and yellow stain in an unexposed portion.

### Example 10

The same tests as in Example 6, test Mo. 69 were repeated provided for replacing the color developing agent in the color developing solution used in Example 6, test No. 69 (Examplary No. X-2) with the hydrochlorides (D-1) and (D-2) shown below. Further, similar tests were carried out by replacing the color developing agent (X-2) with a sulfate of (X-1), p-toluenesulfonate of (X-4) and p-toluenesulfonate of (X-11).

In the above test, the bleaching solution was added with the above color developing solution by 35 % based on the total amount of the bleaching soluiton, respectively and the processing was carried out after storing for one week at a room temperature. A residual silver amount and a magenta stain (bleaching stain) of the film samples after the processing were determined and a generation of tar in the bleaching soluiton was observed. The results are shown in Table 8.

In Table 8, o represents no generation of tar, A represents a little generation of tar and x represents generation of tar to such a degree that a tar adhered to a film.

From Table 8, there are found that, by using the color developing agent according to the present invention, desilvering property, bleaching stain and generation of tar are all improved.

### Example 11

Example 1 was repeated provided for replacing (ethylenediaminetetraacetato) iron (III) complex salt used for the bleaching solution and bleach-fixing solution in Example 1 with iron (III) complex salt of the Examplary compound (XII-4) (1,3-diaminopropanetetraacetate). It was found that a residual silver amount did not genarated at all, 0 mg/100 cm², namely, the property against the residual silver amount was further improved.

Further, the similar experient was carried out by arranging the total added amount in terms of iron salt to 0.37 mole and the mixture ratio of (ethylenediaminetetraacetato) iron (III) complex salt and an iron (III) complex salt of Examplary compound (XII-4) to 1:1 to 2:1. It was also found that a residual silver amount did not genarated at all.

## Claims (Claims for the following Contracting State(s) : DE)

1. A method for processing a light-sensitive silver halide color photographic material having at least one silver halide emulsion layer which comprises subjecting to image-like exposure and subsequently to processing including at least color development step and bleaching step, wherein a bleaching solution employed in said bleaching step contains at least one organic acid ferric complex; and said bleaching solution contains at least one organic acid and said bleaching solution is replenished, characterized in that a light-sensitive silver halide color photographic material is processed wherein at least one layer of said silver halide emulsion layer contains at least one magenta coupler having the general formula (M): wherein Z represents a non-metal atom group necessary to form a nitrogen-containing heterocyclic ring, said ring optionally having a substituent; X represents a hydrogen atom or a substituent eliminable through a reaction with an oxidized product of a color developing agent; and R represents a hydrogen atom or a substituent; that the organic acid is contained in a range of not more than 10 mole % of the content of said organic acid ferric complex contained in said bleaching solution; and that the replenished amount in said bleaching step is 30 mî to 300 mî per 1m² of said silver halide color photographic material.

2. The method for processing a light-sensitive silver halide color photographic material as claimed in claim 1, wherein said bleaching solution contains at least one of the compounds having the under-mentioned general formulae (I) to (IX); wherein Q represents a group of atoms necessary for the formation of a nitrogen-containing heterocyclic ring (including the ring condensed with an unsaturated 5- to 6-membered ring); and R represents a hydrogen atom, an alkyl group having 1 to 6 carbon atoms, a cycloalkyl group, an aryl group, a heterocyclic ring (including the ring condensed with an unsaturated 5- to 6-membered ring) or an amino group, wherein R₂ and R₃ each represent a hydrogen atom, an alkyl group having 1 to 6 carbon atoms, a hydroxyl group, a carboxyl group, an amino group, an acyl group having 1 to 3 carbon atoms, an aryl group or an alkenyl group; A represents: or an n -valent heterocyclic residual group (including the group condensed with an unsaturated 5- to 6- membered ring); X represents = S, = 0 or = NR"; R and R' each have the same meaning as defined for R₂ and R₃; X' has the same meaning as defined for X; Z represents a hydrogen atom, an alkali metal atom, an ammonium group, an amino group, a nitrogen-containing heterocyclic residual group, an alkyl group or M represents a divalent metallic atom; R" represents a hydrogen atom, an alkyl group having 1 to 6 carbon atoms, a cycloalkyl group, an aryl group, a heterocyclic residual group (including the group condensed with an unsaturated 5- to 6-membered ring) or an amino group; and n1 to n6 and m1 to m5 each represent an integer of 1 to 6; B represents an alkylene group having 1 to 6 carbon atoms; Y represents -N or -CH 〈 ; R₄ and R₅ each have the same meaning as defined for R₂ and R₃; provided that R₄ and R₅ each may represent -B-SZ and that R₂ and R₃, R and R', and R₄ and R₅ each may be combined to form a ring, wherein R₆ and R₇ each represent a hydrogen atom, an alkyl group having 1 to 6 carbon atoms, a hydroxyl group, a carboxyl group, an amino group, an acyl group having 1 to 3 carbon atoms, an aryl group, an alkenyl group or -B₁-S-Z₁; provided that R₆ and R₇ may be combined to form a ring; Y₁ represents N- or CH-; B₁ represents an alkylene group having 1 to 6 carbon atoms; Z₁ represents a hydrogen atom, an alkali metal atom, an ammonium group, an amino group, a nitrogen-containing heterocyclic residual group or and n7 represents an integer of 1 to 6, wherein R₈ and R₉ each represent ; and R₁₀ represents an alkyl group or -(CH₂)ₙ₈SO₃^{⊖} (provided that ℓ represents 0 when R₁₀ is -(CH₂)-ₙ₈SO₃⊖, or 1 when it is an alkyl group); G^{⊖} represents an anion; and n8 represents an integer of 1 to 6, wherein Q₁ represents a group of atoms necessary for the formation of a nitrogen-containing heterocyclic ring (including the ring condensed with an unsaturated or saturated 5- to 6-membered ring); and R₁₁ represents a hydrogen atom, an alkali metal atom, or an alkyl group; provided that Q' have the same meaning as defined for Qi, wherein Di, D₂, D₃ and D₄ each represent a simple bond arm, an alkylene group having 1 to 8 carbon atoms or a vinylene group; and q1, q2, q3 and q4 each represent an integer of 0, 1 or 2, said ring formed together with a sulfur atom may be further condensed with a saturated or unsaturated 5- to 6-membered ring, with the exception of elementary sulfur; wherein X₂ represents -COOM', -OH, -SO₃M', -CONH₂, -S0₂NH₂, -NH₂, -SH, -CN, -CO₂R₁₆, -SO₂R₁₆, -OR₁₆, -NR₁₆R₁₇, -SR₁₆, -SO₃R₁₆, -NHCOR₁₆, -NHSO₂R₁₆, -OCOR₁₆ or -SO₂ R₁₆; Y₂ represents or a hydrogen atom; and m9 and n9 each represent an integer of 1 to 10; R₁₁, R12, R₁₃ , R₁₄, R,₁₅, R₁₇ and R₁₈ each represent a hydrogen atom, a lower alkyl group, an acyl group or
R₁₆ represents a lower alkyl group;
R₁₉ represents -NR₂₀R₂₁, -OR₂₂ or -SR₂₂; R₂₀ and R₂₁ each represent a hydrogen atom or a lower alkyl group; and R₂₂ represents a group of atoms necessary for a ring to be formed by combination with R₁₈; R₂₀ or R₁₁ may be combined with R₁₈ to form a ring; M' represents a hydrogen atom or a cation, wherein Ar represents a divalent aryl group or a divalent organic group formed by combination of an aryl group with an oxygen atom and/or alkylene group; B₂ and B₃ each represent a lower alkylene group; R₂₃, R₂₄, R₂₅ and R₂₆ each represent a hydroxyl substituted lower alkyl group; and x and y each represent 0 or 1; G' represents an anion; and z represents 0, 1 or 2, wherein R₂₉ and R₃₀ each represent a hydrogen atom, an alkyl group, an aryl group or a heterocyclic group; R₃, represents a hydrogen atom or an alkyl group; R₃₂ represents a hydrogen atom or a carboxyl group.

3. The method for processing a light-sensitive silver halide color photographic material as claimed in claim 1 or 2 wherein at least one layer of said light-sensitive silver halide color photographic material contains a cyan coupler having the general formula (C): wherein R₂, represents an alkyl group, an alkenyl group, a cycloalkyl group, an aryl group or a heterocyclic group; R₂₄ represents an unsubstituted or substituted aryl group; and Z represents a hydrogen atom or a group iliminatable through coupling reaction with an oxidizing product of a N-hydroxyalkyl substituted-p-phenylenediamine derivative developing agent.

4. The method for processing a light-sensitive silver halide color photographic material as claimed in claim 1, 2 or 3, wherein at least one of the substituents in general formula (M) represents an aromatic sulfonyl group represented by the following formula (A) wherein R represents an aliphatic group, an aryl group or a heterocyclic group; m represents an integer of 1 or 2, R₁ may be identical or different when m is 2; R₂ represents an aliphatic group, an aryl group, a heterocyclic group or where R₃ and R₄ each represent a hydrogen atom, an aliphatic group or an aryl group.

5. The method for processing a light-sensitive silver halide color photographic material as claimed in any of claims 1 to 4, wherein the organic acid or organic acid capable of forming the organic acid ferric complex is a compound represented by the following general formulae (XII) or (XIII): wherein E represents a substituted or unsubstituted alkylene group, a cycloalkylene group, a phenylene group, -R₈₃0R₈₃0R₈₃- or -R₈₃ZR₈₃-, Z represents N-R₈₃-A₆ or N-A₆, R₇₉ to R₈₃ individually represent a substituted or unsubstituted alkylene group, A₂ to A₆ individually represent a hydrogen atom, -OH, -COOM or -P0₃M₂ and M is a hydrogen atom or an alkali metal atom.

6. The method for processing a light-sensitive silver halide color photographic material as claimed in claim 5, wherein said compound represented by the formula (XII) or (XIII) is a compound selected from the group consisting of:
(XII - 1) Ethylenediaminetetraacetic acid
(XII - 2) Diethylenetriaminepentaacetic acid
(XII - 4) Propylenediaminetetraacetic acid
(XII - 5) Triethylenetetraminehexaacetic acid
(XII - 7) 1,2-Diaminopropanetetraacetic acid
(XII - 8) 1,3-Diaminopropan-2-ol-tetraacetic acid
(XII - 19) Ethylenediaminetetramethylene phosphonic acid
(XIII - 1) Nitrilotriacetic acid
(XIII - 3) Hydroxyethyliminodiacetic acid
(XIII - 5) Nitrilotrimethylene phosphonic acid

7. The method for processing a light-sensitive silver halide color photographic material as claimed in any of claims 1 to 6 wherein an amount of the bleaching solution to be replenished is 40 mℓ to 250 mℓ per 1 m² of the light-sensitive silver halide color photographic material.

8. The method for processing a light-sensitive silver halide color photographic material as claimed in claim 7, wherein an amount of the bleaching solution to be replenished is 50 mℓ to 200 mℓ per 1 m² of the light-sensitive silver halide color photographic material.

9. The method for processing a light-sensitive silver halide color photographic material as claimed in claim 2, wherein the bleaching solution contains at least one selected from the group consisting of the compounds represented by the formulae (II), (III), (V) or (VII).

10. The method for processing a light-sensitive silver halide color photographic material as claimed in any of claims 1 to 9 wherein a color developing solution used for the color development step contains a color developing agent represented by the following formula (X): wherein R represents a hydrogen atom, a halogen atom, or an alkyl group, said alkyl group having a straight or branched chain of 1 to 5 carbon atoms and optionally a substituent; R₁₄ and R₁₅ individually represent a hydrogen atom, an alkyl group or an aryl group, said alkyl or aryl group being optionally substituted; at least one of R₁₄ and R₁₅ is an alkyl group substituted with a water-soluble group such as a hydroxy group, a carboxy group, a sulfonic acid group, an amino group, a sulfonamido group or said alkyl group being optionally further substituted; R₁₆ represents a hydrogen atom or an alkyl group having a straight or branched chain of 1 to 5 carbon atoms and p and q each is an integer of 1 to 5.

11. The method for processing a light-sensitive silver halide color photographic material as claimed in any of claims 1 to 10 wherein the light-sensitive silver halide photographic material contains at least one of the compounds having the following general formula (XI): wherein Z₁₁ and Z₂₁ individually represent atom groups required for forming a benzene or naphthalene ring condensed to an oxazole ring; R₄₁ and R₄₂ individually represent an alkyl group, an alkenyl group, or an aryl group, R₄₃ represents a hydrogen atom or an alkyl group having 1 to 3 carbon atoms, X₁⊖ represents an anion, and n is 1 or 0.

## Claims (Claims for the following Contracting State(s) : GB)

1. A method for processing a light-sensitive silver halide color photographic material having at least one silver halide emulsion layer which comprises subjecting to image-like exposure and subsequently to processing including at least color development step and bleaching step, wherein a bleaching solution employed in said bleaching step contains at least one organic acid ferric complex; and said bleaching solution contains at least one organic acid and said bleaching solution is replenished, characterized in that a light-sensitive silver halide color photographic material is processed wherein at least one layer of said silver halide emulsion layer contains at least one magenta coupler having the general formula (M): wherein Z represents a non-metal atom group necessary to form a nitrogen-containing heterocyclic ring, said ring optionally having a substituent; X represents a hydrogen atom or a substituent eliminable through a reaction with an oxidized product of a color developing agent; and R represents a hydrogen atom or a substituent; that the organic acid is contained in a range of not more than 10 mole % of the content of said organic acid ferric complex contained in said bleaching solution; and that the replenished amount in said bleaching step is 30 mî to 300 mî per 1m² of said silver halide color photographic material, with the proviso that the magenta coupler of formula is excepted from the magenta couplers of the general formula (M).

2. The method for processing a light-sensitive silver halide color photographic material as claimed in claim 1, wherein said bleaching solution contains at least one of the compounds having the under-mentioned general formulae (I) to (IX); wherein Q represents a group of atoms necessary for the formation of a nitrogen-containing heterocyclic ring (including the ring condensed with an unsaturated 5- to 6-membered ring); and R represents a hydrogen atom, an alkyl group having 1 to 6 carbon atoms, a cycloalkyl group, an aryl group, a heterocyclic ring (including the ring condensed with an unsaturated 5- to 6-membered ring) or an amino group, wherein R₂ and R₃ each represent a hydrogen atom, an alkyl group having 1 to 6 carbon atoms, a hydroxyl group, a carboxyl group, an amino group, an acyl group having 1 to 3 carbon atoms, an aryl group or an alkenyl group; A represents: or an n₁ -valent heterocyclic residual group (including the group condensed with an unsaturated 5- to 6- membered ring); X represents = S, = 0 or = NR"; R and R' each have the same meaning as defined for R₂ and R₃; X' has the same meaning as defined for X; Z represents a hydrogen atom, an alkali metal atom, an ammonium group, an amino group, a nitrogen-containing heterocyclic residual group, an alkyl group or M represents a divalent metallic atom; R" represents a hydrogen atom, an alkyl group having 1 to 6 carbon atoms, a cycloalkyl group, an aryl group, a heterocyclic residual group (including the group condensed with an unsaturated 5- to 6-membered ring) or an amino group; and n1 to n6 and m1 to m5 each represent an integer of 1 to 6; B represents an alkylene group having 1 to 6 carbon atoms; Y represents -N or -CH〈 ; R₄ and R₅ each have the same meaning as defined for R₂ and R₃; provided that R₄ and R₅ each may represent -B-SZ and that R₂ and R₃, R and R', and R₄ and R₅ each may be combined to form a ring, wherein R₆ and R₇ each represent a hydrogen atom, an alkyl group having 1 to 6 carbon atoms, a hydroxyl group, a carboxyl group, an amino group, an acyl group having 1 to 3 carbon atoms, an aryl group, an alkenyl group or -B₁-S-Z₁; provided that R₆ and R₇ may be combined to form a ring; Y₁ represents N- or CH-; B₁ represents an alkylene group having 1 to 6 carbon atoms; Z₁ represents a hydrogen atom, an alkali metal atom, an ammonium group, an amino group, a nitrogen-containing heterocyclic residual group or and n7 represents an integer of 1 to 6, wherein R₈ and R₉ each represent ; and R₁₀ represents an alkyl group or -(CH₂)ₙ8SO₃⊖ (provided that ℓ represents 0 when R₁₀ is -(CH₂)-ₙ₈SO₃⊖, or 1 when it is an alkyl group); G^{⊖} represents an anion; and n8 represents an integer of 1 to 6, wherein Q₁ represents a group of atoms necessary for the formation of a nitrogen-containing heterocyclic ring (including the ring condensed with an unsaturated or saturated 5- to 6-membered ring); and R₁₁ represents a hydrogen atom, an alkali metal atom, or an alkyl group; provided that Q' have the same meaning as defined for Qi, wherein Di, D₂, D₃ and D₄ each represent a simple bond arm, an alkylene group having 1 to 8 carbon atoms or a vinylene group; and q1, q2, q3 and q4 each represent an integer of 0, 1 or 2, said ring formed together with a sulfur atom may be further condensed with a saturated or unsaturated 5- to 6-membered ring, with the exception of elementary sulfur; wherein X₂ represents -COOM', -OH, -SO₃M', -CONH₂, -S0₂NH₂, -NH₂, -SH, -CN, -CO₂ R₁₆, -SO₂ R₁₆, -OR₁₆, -NR₁₆R₁₇, -SR₁₆, -SO₃R₁₆, -NHCOR₁₆, -NHSO₂R₁₆, -OCOR₁₆ or -SO₂ R₁₆; Y₂ represents or a hydrogen atom; and m9 and n9 each represent an integer of 1 to 10; R₁₁, R12, R₁₃, R₁₄, R₁₅, R₁₇ and R₁₈ each represent a hydrogen atom, a lower alkyl group, an acyl group or
R₁₆ represents a lower alkyl group;
R₁₉ represents -NR₂₀R₂₁, -OR₂₂ or -SR₂₂; R₂₀ and R₂₁ each represent a hydrogen atom or a lower alkyl group; and R₂₂ represents a group of atoms necessary for a ring to be formed by combination with R₁₈; R₂₀ or R₁₁ may be combined with R₁₈ to form a ring; M' represents a hydrogen atom or a cation, wherein Ar represents a divalent aryl group or a divalent organic group formed by combination of an aryl group with an oxygen atom and/or alkylene group; B₂ and B₃ each represent a lower alkylene group; R₂₃, R₂₄, R₂₅ and R₂₆ each represent a hydroxyl substituted lower alkyl group; and x and y each represent 0 or 1; G' represents an anion; and z represents 0, 1 or 2, wherein R₂₉ and R₃₀ each represent a hydrogen atom, an alkyl group, an aryl group or a heterocyclic group; R₃, represents a hydrogen atom or an alkyl group; R₃₂ represents a hydrogen atom or a carboxyl group.

3. The method for processing a light-sensitive silver halide color photographic material as claimed in claim 1 or 2 wherein at least one layer of said light-sensitive silver halide color photographic material contains a cyan coupler having the general formula (C): wherein R₂, represents an alkyl group, an alkenyl group, a cycloalkyl group, an aryl group or a heterocyclic group; R₂₄ represents an unsubstituted or substituted aryl group; and Z represents a hydrogen atom or a group iliminatable through coupling reaction with an oxidizing product of a N-hydroxyalkyl substituted-p-phenylenediamine derivative developing agent.

4. The method for processing a light-sensitive silver halide color photographic material as claimed in claim 1, 2 or 3, wherein at least one of the substituents in general formula (M) represents an aromatic sulfonyl group represented by the following formula (A) wherein R represents an aliphatic group, an aryl group or a heterocyclic group; m represents an integer of 1 or 2, R₁ may be identical or different when m is 2; R₂ represents an aliphatic group, an aryl group, a heterocyclic group or where R₃ and R₄ each represent a hydrogen atom, an aliphatic group or an aryl group.

5. The method for processing a light-sensitive silver halide color photographic material as claimed in any of claims 1 to 4, wherein the organic acid or organic acid capable of forming the organic acid ferric complex is a compound represented by the following general formulae (XII) or (XIII): wherein E represents a substituted or unsubstituted alkylene group, a cycloalkylene group, a phenylene group, -R₈₃0R₈₃0R₈₃- or -R₈₃ZR₈₃-, Z represents N-R₈₃-A₆ or N-A₆, R₇₉ to R₈₃ individually represent a substituted or unsubstituted alkylene group, A₂ to A₆ individually represent a hydrogen atom, -OH, -COOM or -P0₃M₂ and M is a hydrogen atom or an alkali metal atom.

6. The method for processing a light-sensitive silver halide color photographic material as claimed in claim 5, wherein said compound represented by the formula (XII) or (XIII) is a compound selected from the group consisting of:
(XII - 1) Ethylenediaminetetraacetic acid
(XII - 2) Diethylenetriaminepentaacetic acid
(XII - 4) Propylenediaminetetraacetic acid
(XII - 5) Triethylenetetraminehexaacetic acid
(XII - 7) 1,2-Diaminopropanetetraacetic acid
(XII - 8) 1,3-Diaminopropan-2-ol-tetraacetic acid
(XII - 19) Ethylenediaminetetramethylene phosphonic acid
(XIII - 1) Nitrilotriacetic acid
(XIII - 3) Hydroxyethyliminodiacetic acid
(XIII - 5) Nitrilotrimethylene phosphonic acid

7. The method for processing a light-sensitive silver halide color photographic material as claimed in any of claims 1 to 6 wherein an amount of the bleaching solution to be replenished is 40 mî to 250 mℓ per 1 m² of the light-sensitive silver halide color photographic material.

8. The method for processing a light-sensitive silver halide color photographic material as claimed in claim 7, wherein an amount of the bleaching solution to be replenished is 50 mℓ to 200 mℓ per 1 m² of the light-sensitive silver halide color photographic material.

9. The method for processing a light-sensitive silver halide color photographic material as claimed in claim 2, wherein the bleaching solution contains at least one selected from the group consisting of the compounds represented by the formulae (II), (III), (V) or (VII).

10. The method for processing a light-sensitive silver halide color photographic material as claimed in any of claims 1 to 9 wherein a color developing solution used for the color development step contains a color developing agent represented by the following formula (X): wherein R₁₃ represents a hydrogen atom, a halogen atom, or an alkyl group, said alkyl group having a straight or branched chain of 1 to 5 carbon atoms and optionally a substituent; R₁₄ and R₁₅ individually represent a hydrogen atom, an alkyl group or an aryl group, said alkyl or aryl group being optionally substituted; at least one of R₁₄ and R₁₅ is an alkyl group substituted with a water-soluble group such as a hydroxy group, a carboxy group, a sulfonic acid group, an amino group, a sulfonamido group or said alkyl group being optionally further substituted; R₁₆ represents a hydrogen atom or an alkyl group having a straight or branched chain of 1 to 5 carbon atoms and p and q each is an integer of 1 to 5.

11. The method for processing a light-sensitive silver halide color photographic material as claimed in any of claims 1 to 10 wherein the light-sensitive silver halide photographic material contains at least one of the compounds having the following general formula (XI): wherein Z11 and Z₂₁ individually represent atom groups required for forming a benzene or naphthalene ring condensed to an oxazole ring; R₄₁ and R₄₂ individually represent an alkyl group, an alkenyl group, or an aryl group, R₄₃ represents a hydrogen atom or an alkyl group having 1 to 3 carbon atoms, X, represents an anion, and n is 1 or 0.

## Patentansprüche (Patentansprüche für folgende(n) Vertragsstaat(en) : DE)

1. Verfahren zur Herstellung eines lichtempfindlichen farbfotografischen Silberhalogenidmaterials mit wenigstens einer Silberhalogenid-Emulsionsschicht, die einer Bild-artigen Belichtung und einer nachfolgenden Behandlung unterzogen wird, die wenigstens eine Farbentwicklungsstufe und eine Bleichstufe einschließt, worin eine in der Bleichstufe verwendete Bleichlösung wenigstens einen Eisen(III)-komplex einer organischen Säure enthält; und wobei die Bleichlösung wenigstens eine organische Säure enthält und die Bleichlösung nachgefüllt wird, dadurch gekennzeichnet, daß ein lichtempfindliches farbfotografisches Silberhalogenidmaterial behandelt wird, worin wenigstens eine Schicht der Silberhalogenid-Emulsionsschicht wenigstens einen Magenta-Kuppler enthält, der die allgemeine Formel (M) hat worin Z eine Nichtmetall-Atomgruppe ist, die erforderlich ist zur Bildung eines Stickstoff-enthaltenden heterocyclischen Ringes, wobei der Ring gegebenenfalls einen Substituenten hat; X ist ein Wasserstoffatom oder ein durch eine Reaktion mit einem oxidierten Produkt eines Farbentwicklungsmittels eliminierbarer Substituent; und R ist ein Wasserstoffatom oder ein Substituent; daß die organische Säure in einem Bereich von nicht mehr als 10 Mol-% des Gehaltes des Eisen(III)komplexes der organischen Säure enthalten ist, der in der Bleichlösung enthalten ist; und daß die Nachfüllmenge in der Bleichstufe 30 ml bis 300 ml pro 1 m² des farbfotografischen Silberhalogenidmaterials beträgt.

2. Verfahren zur Herstellung eines lichtempfindlichen farbfotografischen Silberhalogenidmaterials nach Anspruch 1, worin die Bleichlösung wenigstens eine der Verbindungen enthält, die die unten aufgeführten allgemeinen Formeln (I) bis (IX) haben; worin Q eine Gruppe von Atomen darstellt, die für die Bildung eines stickstoffhaltigen heterocyclischen Ringes (einschließlich des Ringes, der mit einem ungesättigten 5-bis 6-gliedrigen Ring kondensiert ist) erforderlich ist; und R ist ein Wasserstoffatom, eine Alkylgruppe mit 1 bis 6 Kohlenstoffatomen, eine Cycloalkylgruppe, eine Arylgruppe, ein heterocyclischer Ring (einschließlich des Ringes, der mit einem ungesättigten 5-bis 6-gliedrigen Ring kondensiert ist) oder eine Aminogruppe, worin R₂ und R₃ jeweils ein Wasserstoffatom, eine Alkylgruppe mit 1 bis 6 Kohlenstoffatomen, eine Hydroxygruppe, eine Carboxygruppe, eine Aminogruppe, eine Acylgruppe mit 1 bis 3 Kohlenstoffatomen, eine Arylgruppe oder eine Alkenylgruppe darstellen; A stellt dar oder eine ni -valente heterocyclische Restgruppe (einschließlich der Gruppe, die mit einem ungesättigten 5-bis 6-gliedrigen Ring kondensiert ist); X stellt dar = S, = 0 oder = NR"; R und R' haben jeweils die gleiche Bedeutung, wie sie für R₂ und R₃ definiert ist; X' hat die gleiche Bedeutung, wie für X definiert; Z ist ein Wasserstoffatom, ein Alkalimetallatom, eine Ammoniumgruppe, eine Aminogruppe, eine Stickstoff-enthaltende heterocyclische Restgruppe, eine Alkylgruppe oder
M ist ein zweiwertiges Metallatom;
R" ist ein Wasserstoffatom, eine Alkylgruppe mit 1 bis 6 Kohlenstoffatomen, eine Cycloalkylgruppe, eine Arylgruppe, eine heterocyclische Restgruppe (einschließlich der Gruppe, die mit einem ungesättigten 5-bis 6-gliedrigen Ring kondensiert ist) oder eine Aminogruppe; und n1 bis n6 und m1 bis m5 stellen jeweils eine ganze Zahl von 1 bis 6 dar; B ist eine Alkylengruppe mit 1 bis 6 Kohlenstoffatomen; Y ist -N ( oder -CH ( ; R4 und R₅ haben jeweils die gleiche Bedeutung, wie sie für R₂ und R₃ definiert ist; mit der Maßgabe, daß R₄ und R₅ jeweils -B-SZ darstellen und daß R₂ und R₃, R und R' sowie R₄ und R₅ jeweils zur Bildung eines Ringes kombiniert werden können; worin R₆ und R₇ jeweils ein Wasserstoffatom, eine Alkylgruppe mit 1 bis 6 Kohlenstoffatomen, eine Hydroxygruppe, eine Carboxygruppe, eine Aminogruppe, eine Acylgruppe mit 1 bis 3 Kohlenstoffatomen, eine Arylgruppe, eine Alkenylgruppe oder -B₁-S-Z₁ repräsentieren; mit der Maßgabe, daß R₆ und R₇ zur Bildung eines Ringes vereinigt werden können; Y₁ stellt N-oder CH- dar; B₁ ist eine Alkylengruppe mit 1 bis 6 Kohlenstoffatomen; Z₁ ist ein Wasserstoffatom, ein Alkalimetallatom, eine Ammoniumgruppe, eine Aminogruppe, eine Stickstoff-enthaltende heterocyclische Restgruppe oder und n 7 ist eine ganze Zahl von 1 bis 6; worin R₈ und R₉ jeweils darstellen ; und R₁₀ ist eine Alkylgruppe oder -(CH₂)ₙ₈SO- (vorausgesetzt, daß 1 Null darstellt, wenn R₁₀ die Bedeutung -(CH₂)ₙ₈SO- hat, oder 1 darstellt, wenn es eine Alkylgruppe ist). G- ist ein Anion; und n8 ist eine ganze Zahl von 1 bis 6; worin Q₁ eine Gruppe von Atomen bedeutet, die für die Bildung eines stickstoffhaltigen heterocyclischen Ringes erforderlich ist (einschließlich des Ringes, der mit einem ungesättigten oder gesättigten 5-bis 6-gliedrigen Ring kondensiert ist); und R₁₁ ist ein Wasserstoffatom, ein Alkalimetallatom, oder eine Alkylgruppe; mit der Maßgabe, daß Q' die gleiche Bedeutung wie für Q₁ definiert hat; worin Di, D₂, D₃ und D₄ jeweils einen einfachen Bindungsarm, eine Alkylengruppe mit 1 bis 8 Kohlenstoffatom oder eine Vinylengruppe darstellen; und q1, q2, q3 und q4 sind jeweils eine ganze Zahl 0, 1 oder 2, wobei der zusammen mit einem Schwefelatom gebildete Ring weiterhin mit einem gesättigten oder ungesättigten 5-bis 6-gliedrigen Ring kondensiert sein kann, mit Ausnahme von elementarem Schwefel; worin X₂ darstellt -COOM', -OH, -SO₃M', -CONH₂, -S0₂NH₂, -NH₂, -SH, -CN, -C0₂R₁₆, -SO₂R₁₆, -OR₁₆, -NR₁₆R₁₇, -SR₁₆, -SO₃R₁₆, -NHCOR₁₆, -NHSO₂ R₁₆, -OCOR₁₆ oder -SO₂ R₁₆; Y₂ bedeutet oder ein Wasserstoffatom; und m9 und n9 sind jeweils eine ganze Zahl von 1 bis 10; R₁₁, R₁₂, R₁₃, R₁₄, R₁₅, R₁₇ und R₁₈ sind jeweils ein Wasserstoffatom, eine niedere Alkylgruppe, eine Acylgruppe oder R₁₆ ist eine niedere Alkylgruppe; R₁₉ stellt dar -NR₂₀ R₂₁, -OR₂₂ oder -SR₂₂; R₂₀ und R₂₁ sind jeweils ein Wasserstoffatom oder eine niedere Alkylgruppe; und R₂₂ ist eine Gruppe von Atomen, die für die Bildung eines Ringes in Kombination mit R₁₈ erforderlich ist; R₂₀ oder R₁₁ können mit R₁₈ zur Bildung eines Ringes kombiniert sein; M' ist ein Wasserstoffatom oder ein Kation, worin Ar eine zweiwertige Arylgruppe oder eine zweiwertige organische Gruppe ist, gebildet durch Kombination einer Arylgruppe mit einem Sauerstoffatom und/oder einer Alkylengruppe; B₂ und B₃ sind jeweils eine niedere Alkylengruppe; R₂₃, R₂₄, R₂₅ und R₂₆ stellen jeweils eine Hydroxy-substituierte niedere Alkylgruppe dar; und x und y sind jeweils 0 oder 1; G' ist ein Anion; und z ist 0, 1 oder 2, worin R₂₉ und R₃₀ jeweils ein Wasserstoffatom, eine Alkylgruppe, eine Arylgruppe oder eine heterocyclische Gruppe darstellen; R₃₁ stellt ein Wasserstoffatom oder eine Alkylgruppe dar; R₃₂ stellt ein Wasserstoffatom oder eine Carboxygruppe dar.

3. Verfahren zur Herstellung eines lichtempfindlichen farbfotografischen Silberhalogenidmaterials nach Anspruch 1 oder 2, worin wenigstens eine Schicht des lichtempfindlichen farbfotografischen Silberhalogenidmaterials einen Cyan-Kuppler enthält, der die allgemeine Formel (C) hat: worin R₂₁ eine Alkylgruppe, eine Alkenylgruppe, eine Cycloalkylgruppe, eine Arylgruppe oder eine heterocyclische Gruppe darstellt; R₂₄ ist eine unsubstituierte oder substituierte Arylgruppe; und Z ist ein Wasserstoffatom oder eine Gruppe, die durch eine Kupplungsreaktion mit einem oxidierenden Produkt eines N-Hydroxyalkyl-substituiert-p-phenylendiamin-Derivates als Entwicklungsmittel eliminierbar ist.

4. Verfahren zur Herstellung eines lichtempfindlichen farbfotografischen Silberhalogenidmaterials nach Anspruch 1, 2 oder 3, worin wenigstens einer der Substituenten in der allgemeinen Formel (M) eine aromatische Sulfonylgruppe ist, repräsentiert durch die folgende Formel (A) worin R eine aliphatische Gruppe, eine Arylgruppe oder eine heterocyclische Gruppe darstellt; m ist eine ganze Zahl 1 oder 2, worin R gleich oder verschieden sein kann, wenn m die Bedeutung 2 hat; R₂ ist eine aliphatische Gruppe, eine Arylgruppe eine heterocyclische Gruppe oder wenn R₃ und R₄ jeweils ein Wasserstoffatom, eine aliphatische Gruppe oder eine Arylgruppe darstellen.

5. Verfahren zur Herstellung eines lichtempfindlichen farbfotografischen Silberhalogenidmaterials nach einem der Ansprüche 1 bis 4, worin die organische Säure oder die zur Bildung des Eisen(III)komplexes der organischen Säure fähige organische Säure eine Verbindung ist, die durch die folgenden allgemeinen Formeln (XII) oder (XIII) repräsentiert wird: worin E eine substituierte oder unsubstituierte Alkylengruppe, eine Cycloalkylengruppe, eine Phenylengruppe, -R₈₃0R₈₃0R₈₃- oder -R₈₃ZR₈₃-, Z ist N-R₈₃-A₆ oder N-A₆ bedeutet, R₇₉ bis R₈₃ stellen einzeln eine substituierte oder unsubstituierte Alkylengruppe dar, A₂ bis A₆ stellen einzeln ein Wasserstoffatom, -OH, -COOM oder -P0₃M₂ dar, und M ist ein Wasserstoffatom oder ein Alkalimetallatom.

6. Verfahren zur Herstellung eines lichtempfindlichen farbfotografischen Silberhalogenidmaterials nach Anspruch 5, worin die Verbindung, die durch die Formel (XII) oder (XIII) repräsentiert wird, eine Verbindung ist, die aus der Gruppe ausgewählt ist, bestehend aus:
(XII-1) Ethylendiamintetraessigsäure
(XII-2) Diethylentriaminpentaessigsäure
(XII-4) Propylendiamintetraessigsäure
(XII-5) Triethylentetraminhexaessigsäure
(XII-7) 1,2-Diaminopropantetraessigsäure
(XII-8) 1,3-Diaminopropan-2-ol-tetraessigsäure
(XII-19) Ethylendiamintetraethylenphosphonsäure
(XIII-1) Nitrilotriessigsäure
(XIII-3) Hydroxyethylimino-di-essigsäure
(XIII-5) Nitrilotrimethylenphosphonsäure.

7. Verfahren zur Herstellung eines lichtempfindlichen farbfotografischen Silberhalogenidmaterials nach einem der Ansprüche 1 bis 6, worin die Menge der Bleichlösung, die aufzufüllen ist, 40 ml bis 250 ml pro 1 m² des lichtempfindlichen farbfotografischen Silberhalogenidmaterials beträgt.

8. Verfahren zur Herstellung eines lichtempfindlichen farbfotografischen Silberhalogenidmaterials nach Anspruch 7, worin die Menge der aufzufüllenden Bleichlösung 50 ml bis 200 ml pro 1 m² des lichtempfindlichen farbfotografischen Silberhalogenidmaterials beträgt.

9. Verfahren zur Herstellung eines lichtempfindlichen farbfotografischen Silberhalogenidmaterials nach Anspruch 2, worin die Bleichlösung wenigstens eine Verbindung enthält, ausgewählt aus der Gruppe, die aus den durch die Formeln (11), (111), (V) oder (VII) repräsentierten Verbindungen besteht.

10. Verfahren zur Herstellung eines lichtempfindlichen farbfotografischen Silberhalogenidmaterials nach einem der Ansprüche 1 bis 9, worin eine Farbentwicklungslösung, die für die Farbentwicklungsstufe verwendet wird, ein Farbentwicklungsmittel enthält, das durch die folgende Formel (X) repräsentiert wird: worin R₁₃ ein Wasserstoffatom, ein Halogenatom oder eine Alkylgruppe ist, wobei die Alkylgruppe eine gerade oder verzweigte Kette mit 1 bis 5 Kohlenstoffatomen und gegebenenfalls einem Substituenten hat; R₁₄ und R₁₅ stellen einzeln ein Wasserstoffatom, eine Alkylgruppe oder eine Arylgruppe dar, wobei die Alkyl- oder Arylgruppe gegebenenfalls substituiert sein kann; wenigstens einer der Reste R₁₄ und R₁₅ ist eine Alkylgruppe, die mit einer wasserlöslichen Gruppe substituiert ist, wie einer Hydroxygruppe, einer Carboxygruppe, einer Sulfonsäuregruppe, einer Aminogruppe, einer Sulfonamidogruppe oder mit -[-(CH₂)_{q}-O-]ₚ R₁₆ , wobei die Alkylgruppe gegebenenfalls weiterhin substituiert ist; R₁₆ ist ein Wasserstoffatom oder eine Alkylgruppe mit einer geraden oder verzweigten Kette mit 1 bis 5 Kohlenstoffatomen, und p und q sind jeweils eine ganze Zahl von 1 bis 5.

11. Verfahren zur Herstellung eines lichtempfindlichen farbfotografischen Silberhalogenidmaterials nach einem der Ansprüche 1 bis 10, worin das lichtempfindliche fotografische Silberhalogenidmaterial wenigstens eine der Verbindungen enthält, die die allgemeine Formel (XI) haben: worin Z11 und Z₂₁ jeweils eine Gruppe von Atomen darstellen, die zur Bildung eines Benzenringes oder eines Naphthalenringes, der mit einem Oxazolring kondensiert ist, erforderlich ist; R₄₁ und R₄₂ stellen einzeln eine Alkylgruppe, eine Alkenylgruppe oder eine Arylgruppe dar, R₄₃ ist ein Wasserstoffatom oder eine Alkylgruppe mit 1 bis 3 Kohlenstoffatomen, X, - ist ein Anion und n ist 1 oder 0.

## Patentansprüche (Patentansprüche für folgende(n) Vertragsstaat(en) : GB)

1. Verfahren zur Herstellung eines lichtempfindlichen farbfotografischen Silberhalogenidmaterials mit wenigstens einer Silberhalogenid-Emulsionsschicht, die einer Bild-artigen Belichtung und einer nachfolgenden Behandlung unterzogen wird, die wenigstens eine Farbentwicklungsstufe und eine Bleichstufe einschließt, worin eine in der Bleichstufe verwendete Bleichlösung wenigstens einen Eisen(III)-komplex einer organischen Säure enthält; und wobei die Bleichlösung wenigstens eine organische Säure enthält und die Bleichlösung nachgefüllt wird, dadurch gekennzeichnet, daß ein lichtempfindliches farbfotografisches Silberhalogenidmaterial behandelt wird, worin wenigstens eine Schicht der Silberhalogenid-Emulsionsschicht wenigstens einen Magenta-Kuppler enthält, der die allgemeine Formel (M) hat worin Z eine Nichtmetall-Atomgruppe ist, die erforderlich ist zur Bildung eines Stickstoff-enthaltenden heterocyclischen Ringes, wobei der Ring gegebenenfalls einen Substituenten hat; X ist ein Wasserstoffatom oder ein durch eine Reaktion mit einem oxidierten Produkt eines Farbentwicklungsmittels eliminierbarer Substituent; und R ist ein Wasserstoffatom oder ein Substituent; daß die organische Säure in einem Bereich von nicht mehr als 10 Mol-% des Gehaltes des Eisen(III)komplexes der organischen Säure enthalten ist, der in der Bleichlösung enthalten ist; und daß die Nachfüllmenge in der Bleichstufe 30 ml bis 300 ml pro 1 m² des farbfotografischen Silberhalogenidmaterials beträgt, mit der Maßgabe, daß der Magenta-Kuppler der Formel von den Magenta-Kupplern der allgemeinen Formel (M) ausgenommen ist.

2. Verfahren zur Herstellung eines lichtempfindlichen farbfotografischen Silberhalogenidmaterials nach Anspruch 1, worin die Bleichlösung wenigstens eine der Verbindungen enthält, die die unten aufgeführten allgemeinen Formeln (I) bis (IX) haben; worin Q eine Gruppe von Atomen darstellt, die für die Bildung eines stickstoffhaltigen heterocyclischen Ringes (einschließlich des Ringes, der mit einem ungesättigten 5-bis 6-gliedrigen Ring kondensiert ist) erforderlich ist; und R ist ein Wasserstoffatom, eine Alkylgruppe mit 1 bis 6 Kohlenstoffatomen, eine Cycloalkylgruppe, eine Arylgruppe, ein heterocyclischer Ring (einschließlich des Ringes, der mit einem ungesättigten 5-bis 6-gliedrigen Ring kondensiert ist) oder eine Aminogruppe, worin R₂ und R₃ jeweils ein Wasserstoffatom, eine Alkylgruppe mit 1 bis 6 Kohlenstoffatomen, eine Hydroxygruppe, eine Carboxygruppe, eine Aminogruppe, eine Acylgruppe mit 1 bis 3 Kohlenstoffatomen, eine Arylgruppe oder eine Alkenylgruppe darstellen; A stellt dar oder eine ni -valente heterocyclische Restgruppe (einschließlich der Gruppe, die mit einem ungesättigten 5-bis 6-gliedrigen Ring kondensiert ist); X stellt dar = S, = 0 oder = NR"; R und R' haben jeweils die gleiche Bedeutung, wie sie für R₂ und R₃ definiert ist; X' hat die gleiche Bedeutung, wie für X definiert; Z ist ein Wasserstoffatom, ein Alkalimetallatom, eine Ammoniumgruppe, eine Aminogruppe, eine Stickstoff-enthaltende heterocyclische Restgruppe, eine Alkylgruppe oder
M ist ein zweiwertiges Metallatom;
R" ist ein Wasserstoffatom, eine Alkylgruppe mit 1 bis 6 Kohlenstoffatomen, eine Cycloalkylgruppe, eine Arylgruppe, eine heterocyclische Restgruppe (einschließlich der Gruppe, die mit einem ungesättigten 5-bis 6-gliedrigen Ring kondensiert ist) oder eine Aminogruppe; und n1 bis n6 und m1 bis m5 stellen jeweils eine ganze Zahl von 1 bis 6 dar; B ist eine Alkylengruppe mit 1 bis 6 Kohlenstoffatomen; Y ist -N 〈 oder -CH〈 ; R4 und R₅ haben jeweils die gleiche Bedeutung, wie sie für R₂ und R₃ definiert ist; mit der Maßgabe, daß R₄ und R₅ jeweils -B-SZ darstellen und daß R₂ und R₃, R und R' sowie R₄ und R₅ jeweils zur Bildung eines Ringes kombiniert werden können; allgemeine Formel (III): worin R₆ und R₇ jeweils ein Wasserstoffatom, eine Alkylgruppe mit 1 bis 6 Kohlenstoffatomen, eine Hydroxygruppe, eine Carboxygruppe, eine Aminogruppe, eine Acylgruppe mit 1 bis 3 Kohlenstoffatomen, eine Arylgruppe, eine Alkenylgruppe oder -B₁-S-Z₁ repräsentieren; mit der Maßgabe, daß R₆ und R₇ zur Bildung eines Ringes vereinigt werden können; Y₁ stellt N- oder CH- dar; B₁ ist eine Alkylengruppe mit 1 bis 6 Kohlenstoffatomen; Z₁ ist ein Wasserstoffatom, ein Alkalimetallatom, eine Ammoniumgruppe, eine Aminogruppe, eine Stickstoff-enthaltende heterocyclische Restgruppe oder und n 7 ist eine ganze Zahl von 1 bis 6; worin R₈ und R₉ jeweils darstellen ; und R₁₀ ist eine Alkylgruppe oder -(CH₂)ₙ₈SO-(vorausgesetzt, daß 1 Null darstellt, wenn R₁₀ die Bedeutung -(CH₂)ₙ₈SO- hat, oder 1 darstellt, wenn es eine Alkylgruppe ist). G- ist ein Anion; und n8 ist eine ganze Zahl von 1 bis 6; worin Q₁ eine Gruppe von Atomen bedeutet, die für die Bildung eines stickstoffhaltigen heterocyclischen Ringes erforderlich ist (einschließlich des Ringes, der mit einem ungesättigten oder gesättigten 5-bis 6-gliedrigen Ring kondensiert ist); und R₁₁ ist ein Wasserstoffatom, ein Alkalimetallatom, oder eine Alkylgruppe; mit der Maßgabe, daß Q' die gleiche Bedeutung wie für Q₁ definiert hat; worin Di, D₂, D₃ und D₄ jeweils einen einfachen Bindungsarm, eine Alkylengruppe mit 1 bis 8 Kohlenstoffatom oder eine Vinylengruppe darstellen; und q1, q2, q3 und q4 sind jeweils eine ganze Zahl 0, 1 oder 2, wobei der zusammen mit einem Schwefelatom gebildete Ring weiterhin mit einem gesättigten oder ungesättigten 5-bis 6-gliedrigen Ring kondensiert sein kann, mit Ausnahme von elementarem Schwefel; worin X₂ darstellt -COOM', -OH, -SO₃M', -CONH₂, -S0₂NH₂, -NH₂, -SH, -CN, -C0₂R₁₆, -SO₂R₁₆, -OR₁₆, -NR₁₆R₁₇, -SR₁₆, -SO₃ R₁₆, -NHCOR₁₆, -NHSO₂R₁₆, -OCOR₁₆ oder -SO₂ R₁₆; Y₂ bedeutet oder ein Wasserstoffatom; und m9 und n9 sind jeweils eine ganze Zahl von 1 bis 10; R₁₁, R₁₂, R₁₃, R₁₄, R₁₅, R₁₇ und R₁₈ sind jeweils ein Wasserstoffatom, eine niedere Alkylgruppe, eine Acylgruppe oder R₁₆ ist eine niedere Alkylgruppe; R₁₉ stellt dar -NR₂₀R₂₁, -OR₂₂ oder -SR₂₂; R₂₀ und R₂₁ sind jeweils ein Wasserstoffatom oder eine niedere Alkylgruppe; und R₂₂ ist eine Gruppe von Atomen, die für die Bildung eines Ringes in Kombination mit R₁₈ erforderlich ist; R₂₀ oder R₁₁ können mit R₁₈ zur Bildung eines Ringes kombiniert sein; M' ist ein Wasserstoffatom oder ein Kation, worin Ar eine zweiwertige Arylgruppe oder eine zweiwertige organische Gruppe ist, gebildet durch Kombination einer Arylgruppe mit einem Sauerstoffatom und/oder einer Alkylengruppe; B₂ und B₃ sind jeweils eine niedere Alkylengruppe; R₂₃, R₂₄, R₂₅ und R₂₆ stellen jeweils eine Hydroxy-substituierte niedere Alkylgruppe dar; und x und y sind jeweils 0 oder 1; G' ist ein Anion; und z ist 0, 1 oder 2, worin R₂₉ und R₃₀ jeweils ein Wasserstoffatom, eine Alkylgruppe, eine Arylgruppe oder eine heterocyclische Gruppe darstellen; R₃₁ stellt ein Wasserstoffatom oder eine Alkylgruppe dar; R₃₂ stellt ein Wasserstoffatom oder eine Carboxygruppe dar.

3. Verfahren zur Herstellung eines lichtempfindlichen farbfotografischen Silberhalogenidmaterials nach Anspruch 1 oder 2, worin wenigstens eine Schicht des lichtempfindlichen farbfotografischen Silberhalogenidmaterials einen Cyan-Kuppler enthält, der die allgemeine Formel (C) hat: worin R₂₁ eine Alkylgruppe, eine Alkenylgruppe, eine Cycloalkylgruppe, eine Arylgruppe oder eine heterocyclische Gruppe darstellt; R₂₄ ist eine unsubstituierte oder substituierte Arylgruppe; und Z ist ein Wasserstoffatom oder eine Gruppe, die durch eine Kupplungsreaktion mit einem oxidierenden Produkt eines N-Hydroxyalkyl-substituiert-p-phenylendiamin-Derivates als Entwicklungsmittel eliminierbar ist.

4. Verfahren zur Herstellung eines lichtempfindlichen farbfotografischen Silberhalogenidmaterials nach Anspruch 1, 2 oder 3, worin wenigstens einer der Substituenten in der allgemeinen Formel (M) eine aromatische Sulfonylgruppe ist, repräsentiert durch die folgende Formel (A) worin R eine aliphatische Gruppe, eine Arylgruppe oder eine heterocyclische Gruppe darstellt; m ist eine ganze Zahl 1 oder 2, worin R gleich oder verschieden sein kann, wenn m die Bedeutung 2 hat; R₂ ist eine aliphatische Gruppe, eine Arylgruppe eine heterocyclische Gruppe oder wenn R₃ und R₄ jeweils ein Wasserstoffatom, eine aliphatische Gruppe oder eine Arylgruppe darstellen.

5. Verfahren zur Herstellung eines lichtempfindlichen farbfotografischen Silberhalogenidmaterials nach einem der Ansprüche 1 bis 4, worin die organische Säure oder die zur Bildung des Eisen(III)komplexes der organischen Säure fähige organische Säure eine Verbindung ist, die durch die folgenden allgemeinen Formeln (XII) oder (XIII) repräsentiert wird: worin E eine substituierte oder unsubstituierte Alkylengruppe, eine Cycloalkylengruppe, eine Phenylengruppe, -R₈₃0R₈₃0R₈₃- oder -R₈₃ZR₈₃-, Z ist N-R₈₃-A₆ oder N-A6 bedeutet, R₇₉ bis R₈₃ stellen einzeln eine substituierte oder unsubstituierte Alkylengruppe dar, A₂ bis A₆ stellen einzeln ein Wasserstoffatom, -OH, -COOM oder -P0₃M₂ dar, und M ist ein Wasserstoffatom oder ein Alkalimetallatom.

6. Verfahren zur Herstellung eines lichtempfindlichen farbfotografischen Silberhalogenidmaterials nach Anspruch 5, worin die Verbindung, die durch die Formel (XII) oder (XIII) repräsentiert wird, eine Verbindung ist, die aus der Gruppe ausgewählt ist, bestehend aus:
(XII-1) Ethylendiamintetraessigsäure
(XII-2) Diethylentriaminpentaessigsäure
(XII-4) Propylendiamintetraessigsäure
(XII-5) Triethylentetraminhexaessigsäure
(XII-7) 1,2-Diaminopropantetraessigsäure
(XII-8) 1,3-Diaminopropan-2-ol-tetraessigsäure
(XII-19) Ethylendiamintetraethylenphosphonsäure
(XIII-1) Nitrilotriessigsäure
(XIII-3) Hydroxyethylimino-di-essigsäure
(XIII-5) Nitrilotrimethylenphosphonsäure.

7. Verfahren zur Herstellung eines lichtempfindlichen farbfotografischen Silberhalogenidmaterials nach einem der Ansprüche 1 bis 6, worin die Menge der Bleichlösung, die aufzufüllen ist, 40 ml bis 250 ml pro 1 m² des lichtempfindlichen farbfotografischen Silberhalogenidmaterials beträgt.

8. Verfahren zur Herstellung eines lichtempfindlichen farbfotografischen Silberhalogenidmaterials nach Anspruch 7, worin die Menge der aufzufüllenden Bleichlösung 50 ml bis 200 ml pro 1 m² des lichtempfindlichen farbfotografischen Silberhalogenidmaterials beträgt.

9. Verfahren zur Herstellung eines lichtempfindlichen farbfotografischen Silberhalogenidmaterials nach Anspruch 2, worin die Bleichlösung wenigstens eine Verbindung enthält, ausgewählt aus der Gruppe, die aus den durch die Formeln (11), (III), (V) oder (VII) repräsentierten Verbindungen besteht.

10. Verfahren zur Herstellung eines lichtempfindlichen farbfotografischen Silberhalogenidmaterials nach einem der Ansprüche 1 bis 9, worin eine Farbentwicklungslösung, die für die Farbentwicklungsstufe verwendet wird, ein Farbentwicklungsmittel enthält, das durch die folgende Formel (X) repräsentiert wird: worin R₁₃ ein Wasserstoffatom, ein Halogenatom oder eine Alkylgruppe ist, wobei die Alkylgruppe eine gerade oder verzweigte Kette mit 1 bis 5 Kohlenstoffatomen und gegebenenfalls einem Substituenten hat; R₁₄ und R₁₅ stellen einzeln ein Wasserstoffatom, eine Alkylgruppe oder eine Arylgruppe dar, wobei die Alkyl- oder Arylgruppe gegebenenfalls substituiert sein kann; wenigstens einer der Reste R₁₄ und R₁₅ ist eine Alkylgruppe, die mit einer wasserlöslichen Gruppe substituiert ist, wie einer Hydroxygruppe, einer Carboxygruppe, einer Sulfonsäuregruppe, einer Aminogruppe, einer Sulfonamidogruppe oder mit -[-(CH₂)_{q}-O-]ₚ-R₁₆,wobei die Alkylgruppe gegebenenfalls weiterhin substituiert ist; R₁₆ ist ein Wasserstoffatom oder eine Alkylgruppe mit einer geraden oder verzweigten Kette mit 1 bis 5 Kohlenstoffatomen, und p und q sind jeweils eine ganze Zahl von 1 bis 5.

11. Verfahren zur Herstellung eines lichtempfindlichen farbfotografischen Silberhalogenidmaterials nach einem der Ansprüche 1 bis 10, worin das lichtempfindliche fotografische Silberhalogenidmaterial wenigstens eine der Verbindungen enthält, die die allgemeine Formel (XI) haben: worin Z₁₁ und Z₂₁ jeweils eine Gruppe von Atomen darstellen, die zur Bildung eines Benzenringes oder eines Naphthalenringes, der mit einem Oxazolring kondensiert ist, erforderlich ist; R₄₁ und R₄₂ stellen einzeln eine Alkylgruppe, eine Alkenylgruppe oder eine Arylgruppe dar, R₄₃ ist ein Wasserstoffatom oder eine Alkylgruppe mit 1 bis 3 Kohlenstoffatomen, X, - ist ein Anion und n ist 1 oder 0.

## Revendications (Revendications pour l'(les) Etat(s) contractant(s) suivant(s) : suivant : DE)

1. Procédé de traitement d'un matériau photographique couleur d'halogénure d'argent photosensible présentant au moins une couche d'émulsion d'halogénure d'argent qui comprend d'exposer à la lumière pour former une image et ensuite de traiter ce qui comprend au moins une étape de traitement chromogène et une étape de blanchiment dans laquelle une solution de blanchiment utilisée lors de ladite étape de blanchiment contient au moins un complexe organique ferrique acide; et ladite solution de blanchiment contient au moins un acide organique et ladite solution de blanchiment est régénérée, caractérisé en ce qu'on traite un matériau photographique couleur d'halogénure d'argent photosensible, dans lequel au moins une couche de ladite émulsion d'halogénure d'argent contient au moins un coupleur magenta ayant la formule générale (M) : dans laquelle Z représente un groupe d'atomes non métalliques nécessaire pour former un cycle hétérocyclique contenant de l'azote, ledit cycle ayant en variante un substituant; X représente un atome d'hydrogène ou un substituant éliminable par réaction avec un produit oxydé d'un agent développeur de couleur; et R représente un atome d'hydrogène ou un substituant; l'acide organique est compris dans un intervalle qui ne dépasse pas 10 % molaire de la teneur dudit complexe ferrique organique acide présent dans ladite solution de blanchiment, la quantité de régénérant à ladite étape de blanchiment est de 30 ml à 300 ml pour 1 m² de matériau photographique couleur d'halogénure d'argent.

2. Procédé de traitement d'un matériau photographique couleur d'halogénure d'argent photosensible selon la revendication 1, dans lequel ladite solution de blanchiment contient au moins l'un des composés ayant les formules générales mentionnées ci-dessous (I) à (IX): dans laquelle Q représente un groupe d'atomes nécessaires à la formation d'un cycle hétérocyclique contenant de l'azote (y compris le cycle condensé avec un cycle insaturé de 5 à 6 membres); et R représente un atome d'hydrogène, un groupe alkyle ayant de 1 à 6 atomes de carbone, un groupe cycloalkyle, un groupe aryle, un cycle hétérocyclique (y compris le cycle condensé avec un cycle insaturé de 5 à 6 membres) ou un groupe amino, dans laquelle R₂ et R₃ représentent chacun un atome d'hydrogène, un groupe alkyle ayant de 1 à 6 atomes de carbone, un groupe hydroxyle, un groupe carboxyle, un groupe amino, un groupe acyle ayant de 1 à 3 atomes de carbone, un groupe aryle ou un groupe alcényle; A représente ou un groupe résiduel hétérocyclique ni -valent (y compris le groupe condensé avec un cycle insaturé de 5 à 6 membres); X représente = S, = 0 ou = NR"; R et R' ont chacun la même signification que celle définie pour R₂ et R₃; X' a la même signification que celle définie pour X; Z représente un atome d'hydrogène, un atome de métal alcalin, un groupe ammonium, un groupe amino, un groupe résiduel hétérocyclique contenant de l'azote, un groupe alkyle ou M représente un atome métallique divalent; R" représente un atome d'hydrogène, un groupe alkyle ayant de 1 à 6 atomes de carbone, un groupe cycloalkyle, un groupe aryle, un groupe résiduel hétérocyclique (y compris le groupe condensé avec un cycle insaturé de 5 ou 6 membres) ou un groupe amino; et n1 à n6 et m1 à m6 représentent chacun un entier de 1 à 6; B représente un groupe alkylène ayant de 1 à 6 atomes de carbone; Y représente -N 〈 ou -CH〈 ; R₄ et R₅ ont chacun la même signification que celle définie pour R₂ et R₃; à la condition que R₄ et R₅ puissent représenter chacun -B-SZ et que R₂ et R₃, R et R', et R₄ et R₅ puissent être combinés chacun pour former un cycle, dans laquelle R₆ et R₇ représentent chacun un atome d'hydrogène, un groupe alkyle ayant de 1 à 6 atomes de carbone, un groupe hydroxyle, un groupe carboxyle, un groupe amino, un groupe acyle ayant 1 à 3 atomes de carbone, un groupe aryle, un groupe alcényle ou -B₁-S-Z₁ ; à la condition que R₆ et R₇ puissent être combinés pour former un cycle; Y₁ représente N- ou CH-; B₁ représente un groupe alkylène ayant de 1 à 6 atomes de carbone; Z₁ représente un atome d'hydrogène, un atome de métal alcalin, un groupe ammonium, un groupe amino, un groupe résiduel hétérocyclique contenant de l'azote ou et n7 représente un entier de 1 à 6, dans laquelle R₈ et R₉ représentent chacun ou ; et R₁₀ représente un groupe alkyle ou -(CH2 )ₙ₈SO₃⊖ (à condition que ℓ représente 0 quand R₁₀ est -(CH₂)ₙ₈SO₃⊖ , ou 1 quand c'est un groupe alkyle); G^{⊖} représente un anion; et n8 représente un entier de 1 à 6, dans laquelle Q₁ représente un groupe d'atomes nécessaire à la formation d'un cycle hétérocyclique contenant de l'azote (y compris le cycle condensé avec un cycle insaturé ou saturé de 5 à 6 membres); et R₁₁ représente un atome d'hydrogène, un atome de métal alcalin, ou un groupe alkyle; à la condition que Q' ait la même signification que celle définie pour Qi, dans laquelle Dᵢ, D₂, D₃ et D₄ représentent chacun une simple liaison, un groupe alkylène ayant de 1 à 8 atomes de carbone ou un groupe vinylène; et q1, q2, q3 et q4 représentent chacun un entier 0, 1 ou 2, ledit cycle formé avec un atome de soufre, peut être encore condensé avec un cycle saturé ou non de 5 à 6 membres, à l'exception du soufre élémentaire; dans laquelle X₂ représente -COOM', -OH, -SO₃M', -CONH₂, -S0₂NH₂, -NH₂, -SH, -CN, -CO₂ R₁₆, -SO₂ R₁₆, -OR₁₆, -NR₁₆R₁₇, -SR₁₆, -SO₃ R₁₆, -NHCOR₁₆, -NHSO₂ R₁₆, -OCOR₁₆ ou -SO₂ R₁₆; Y₂ représente ou un atome d'hydrogène; et m9 et n9 représentent chacun un entier de 1 à 10; R₁₁, R₁₂, R₁₃, R₁₄, R₁₅, R₁₇ et R₁₈ représentent chacun un atome d'hydrogène, un groupe alkyle inférieur, un groupe acyle ou
R₁₆ représente un groupe alkyle inférieur;
R₁₉ représente -NR₂₀R₂₁, -OR₂₂ ou -SR₂₂; R₂₀ et R₂, représentent chacun un atome d'hydrogène ou un groupe alkyle inférieur; et R₂₂ représente un groupe d'atomes nécessaire pour former un cycle en combinaison avec R₁₈; R₂₀ ou R₁₁ peuvent être combinés avec R₁₈ pour former un cycle; M' représente un atome d'hydrogène ou un cation, dans laquelle Ar représente un groupe aryle divalent ou un groupe organique divalent formé par combinaison d'un groupe aryle avec un atome d'oxygène et/ou un groupe alkylène; B₂ et B₃ représentent chacun un groupe alkylène inférieur, R₂₃, R₂₄, R₂₅ et R₂₆ représentent chacun un groupe alkyle inférieur substitué par un hydroxyle; et x et y représentent chacun 0 ou 1; G' représente un anion; et Z représente 0, 1 ou 2, dans laquelle R₂₉ et R₃₀ représentent chacun un atome d'hydrogène, un groupe alkyle, un groupe aryle ou un groupe hétérocyclique; R₃, représente un atome d'hydrogène ou un groupe alkyle; R₃₂ représente un atome d'hydrogène ou un groupe carboxyle.

3. Procédé de traitement d'un matériau photographique couleur d'halogénure d'argent photosensible selon la revendication 1 ou 2, dans lequel au moins une couche dudit matériau photographique couleur d'halogénure d'argent photosensible contient un coupleur cyan de formule générale (C) : dans laquelle R₂₁ représente un groupe alkyle, un groupe alcényle, un groupe cycloalkyle, un groupe aryle ou un groupe hétérocyclique; R₂₄ représente un groupe aryle non substitué ou substitué; et Z représente un atome d'hydrogène ou un groupe éliminable par réaction de couplage avec un produit oxydant d'un agent développeur dérivé de p-phénylènediamine N-hydroxyalkyle substitué.

4. Procédé de traitement d'un matériau photographique couleur d'halogénure d'argent photosensible selon la revendication 1, 2 ou 3, dans lequel au moins l'un des substituants dans formule générale (M) représente un groupe sulfonyle aromatique, représenté par la formule suivante (A) dans laquelle R représente un groupe aliphatique, un groupe aryle ou un groupe hétérocyclique; m représente un entier 1 ou 2, R peut être identique ou différent quand m est 2; R₂ représente un groupe aliphatique, un groupe aryle, un groupe hétérocyclique ou où R₃ et R₄ représentent chacun un atome d'hydrogène, un groupe aliphatique ou un groupe aryle.

5. Procédé de traitement d'un matériau photographique couleur d'halogénure d'argent photosensible selon l'une quelconque des revendications 1 à 4, dans lequel l'acide organique ou l'acide organique capable de former le complexe ferrique organique acide est un composé représenté par les formules générales suivantes (XII) ou (XIII) : dans lesquelles E représente un groupe alkylène substitué ou non substitué, un groupe cycloalkylène, un groupe phénylène, -R₈₃0R₈₃0R₈₃- ou R₈₃ZR₈₃-, Z représente N-R₈₃-A₆ ou N-A₆, R₇₉ à R₈₃ individuellement représentent un groupe alkylène substitué ou non substitué, A₂ à A₆ représentent individuellement un atome d'hydrogène, -OH, -COOM ou PO₃M₂ et M est un atome d'hydrogène ou un atome de métal alcalin.

6. Procédé de traitement d'un matériau photographique couleur d'halogénure d'argent photosensible selon la revendication 5, dans lequel ledit composé représenté par la formule (XII) ou (XIII) est un composé choisi dans le groupe constitué de :
(XII - 1) acide éthylènediaminetétraacétique
(XII - 2) acide diéthylènetriaminepentaacétique
(XII - 4) acide propylènediaminetétraacétique
(XII - 5) acide triéthylènetétraminehexaacétique
(XII - 7) acide 1,2-diaminopropanetétraacétique
(XII - 8) acide 1,3-diaminopropane-2-ol-tétraacétique
(XII - 19) acide éthylènediaminetétraméthylène phosphonique
(XIII - 1) acide nitrilotriacétique
(XIII - 3) acide hydroxyéthyliminodiacétique
(XIII - 5) acide nitrilotriméthylène phosphonique

7. Procédé de traitement d'un matériau photographique couleur d'halogénure d'argent photosensible selon l'une quelconque des revendications 1 à 6, dans laquelle la quantité de solution de blanchiment à régénérer est de 40 ml à 250 ml par 1 m² de matériau photographique couleur d'halogénure d'argent photosensible.

8. Procédé de traitement de matériau photographique couleur d'halogénure d'argent photosensible selon la revendication 7, dans lequel la quantité de solution de blanchiment à régénérer est de 50 ml à 200 ml par 1 m² de matériau photographique couleur d'halogénure d'argent photosensible.

9. Procédé de traitement de matériau photographique couleur d'halogénure d'argent photosensible selon la revendication 2 dans lequel la solution de blanchiment contient au moins l'un des composés choisi dans le groupe constitué des composés représentés par les formules (II), (III), (V) ou (VII).

10. Procédé de traitement d'un matériau photographique couleur d'halogénure d'argent photosensible selon l'une quelconque des revendications 1 à 9, dans lequel on utilise une solution révélatrice de couleur à l'étape du développement de la couleur qui contient un agent développeur de couleur représenté par la formule suivante (X) : dans laquelle R représente un atome d'hydrogène, un atome d'halogène, ou un groupe alkyle, ledit groupe alkyle ayant une chaîne droite ou ramifiée de 1 à 5 atomes de carbone et en option un substituant R₁₄ et R₁₅ représentent individuellement un atome d'hydrogène, un groupe alkyle ou un groupe aryle, ledit groupe alkyle ou aryle étant substitué en variante; au moins l'un des groupes R₁₄ et R₁₅ est un groupe alkyle substitué par un groupe hydrosoluble, tel qu'un groupe hydroxy, un groupe carboxy, un groupe acide sulfonique, un groupe amino, un groupe sulfonamido ou ledit groupe alkyle étant encore substitué en variante; R₁₆ représente un atome d'hydrogène ou un groupe alkyle ayant une chaîne droite ou ramifiée de 1 à 5 atomes de carbone et p et q représentent chacun un entier de 1 à 5.

11. Procédé de traitement d'un matériau photographique couleur d'halogénure d'argent photosensible selon l'une quelconque des revendications 1 à 10 dans lequel le matériau photographique d'halogénure d'argent photosensible contient au moins l'un des composés ayant la formule générale (XI) : dans laquelle Z₁₁ et Z₂, représentent individuellement des groupes d'atomes requis pour former un cycle benzénique ou naphtalénique condensés sur un cycle oxazole; R₄₁ et R₄₂ représentent individuellement un groupe alkyle, un groupe alcényle ou un groupe aryle, R₄₃ représente un atome d'hydrogène ou un groupe alkyle ayant de 1 à 3 atomes de carbone, X, représente un anion et n est 1 ou 0.

## Revendications (Revendications pour l'(les) Etat(s) contractant(s) suivant(s) : suivant : GB)

1. Procédé de traitement d'un matériau photographique couleur d'halogénure d'argent photosensible présentant au moins une couche d'émulsion d'halogéure d'argent qui comprend d'exposer à la lumière pour former une image et ensuite de traiter ce qui comprend au moins une étape de traitement chromogène et une étape de blanchiment dans laquelle une solution de blanchiment utilisée lors de ladite étape de blanchiment contient au moins un complexe organique ferrique acide; et ladite solution de blanchiment contient au moins un acide organique et ladite solution de blanchiment est régénérée, caractérisé en ce qu'on traite un matériau photographique couleur d'halogénure d'argent photosensible, dans lequel au moins une couche de ladite émulsion d'halogénure d'argent contient au moins un coupleur magenta ayant la formule générale (M) : dans laquelle Z représente un groupe d'atomes non métalliques nécessaire pour former un cycle hétérocyclique contenant de l'azote, ledit cycle ayant en variante un substituant; X représente un atome d'hydrogène ou un substituant éliminable par réaction avec un produit oxydé d'un agent développeur de couleur; et R représente un atome d'hydrogène ou un substituant; l'acide organique est compris dans un intervalle qui ne dépasse pas 10 % molaire de la teneur dudit complexe ferrique organique acide présent dans ladite solution de blanchiment , la quantité de régénérant à ladite étape de blanchiment est de 30 ml à 300 ml pour 1 m² de matériau photographique couleur d'halogénure d'argent, à la condition que le coupleur magenta de formule soit exclu des coupleurs magenta de formule générale M.

2. Procédé de traitement d'un matériau photographique couleur d'halogénure d'argent photosensible selon la revendication 1, dans lequel ladite solution de blanchiment contient au moins l'un des composés ayant les formules générales mentionnées ci-dessous (I) à (IX); dans laquelle R représente un groupe d'atomes nécessaires à la formation d'un cycle hétérocyclique contenant de l'azote (y compris le cycle condensé avec un cycle insaturé de 5 à 6 membres), et R représente un atome d'hydrogène, un groupe alkyle ayant de 1 à 6 atomes de carbone, un groupe cycloalkyle, un groupe aryle, un cycle hétérocyclique (y compris le cycle condensé avec un cycle insaturé de 5 à 6 membres) ou un groupe amino, dans laquelle R₂ et R₃ représentent chacun un atome d'hydrogène, un groupe alkyle ayant de 1 à 6 atomes de carbone, un groupe hydroxyle, un groupe carboxyle, un groupe amino, un groupe acyle ayant de 1 à 3 atomes de carbone, un groupe aryle ou un groupe alcényle;
A représente ou un groupe résiduel hétérocyclique ni -valent (y compris le groupe condensé avec un cycle insaturé de 5 à 6 membres); X représente = S, = 0 ou = NR"; R et R' ont chacun la même signification que celle définie pour R₂ et R₃; X' a la même signification que celle définie pour X; Z représente un atome d'hydrogène, un atome de métal alcalin, un groupe ammonium, un groupe amino, un groupe résiduel hétérocyclique contenant de l'azote, un groupe alkyle ou
M représente un atome métallique divalent; R" représente un atome d'hydrogène, un groupe alkyle ayant de 1 à 6 atomes de carbone, un groupe cycloalkyle, un groupe aryle, un groupe résiduel hétérocyclique (y compris le groupe condensé avec un cycle insaturé de 5 ou 6 membres) ou un groupe amino; et n¹ à n⁶et m¹ à m⁶ représentent chacun un entier de 1 à 6; B représente un groupe alkylène ayant de 1 à 6 atomes de carbone; Y représente -N 〈 ou -CH〈 ; R₄ et R₅ ont chacun la même signification que celle définie pour R₂ et R₃; à la condition que R₄ et R₅ puissent représenter chacun -B-SZ et que R₂ et R₃, R et R', et R₄ et R₅ puissent être combinés chacun pour former un cycle, dans laquelle R₆ et R₇ représentent chacun un atome d'hydrogène, un groupe alkyle ayant de 1 à 6 atomes de carbone, un groupe hydroxyle, un groupe carboxyle, un groupe amino, un groupe acyle ayant 1 à 3 atomes de carbone, un groupe aryle, un groupe alcényle ou -B₁-S-Z₁; à la condition que R₆ et R₇ puissent être combinés pour former un cycle; Y₁ représente N ou CH-; B₁ représente un groupe alkylène ayant de 1 à 6 atomes de carbone; Z₁ représente un atome d'hydrogène, un atome de métal alcalin, un groupe ammonium, un groupe amino, un groupe résiduel hétérocyclique contenant de l'azote ou et n₇ représente un entier de 1 à 6, dans laquelle R₈ et R₉ représentent chacun ou ; et R₁₀ représente un groupe alkyle ou -(CH₂)ₙ₈SO₃⊖ (à condition que 1 représente 0 quand R₁₀ est -(CH₂)ₙ₈SO₃^{⊖} , ou 1 quand c'est un groupe alkyle); G⊖ représente un anion; et n8 représente un entier de 1 à 6, dans laquelle Q₁ représente un groupe d'atomes nécessaire à la formation d'un cycle hétérocyclique contenant de l'azote ( y compris le cycle condensé avec un cycle insaturé ou saturé de 5 à 6 membres); et R₁₁ représente un atome d'hydrogène, un atome de métal alcalin, ou un groupe alkyle; à la condition que Q' ait la même signification que celle définie pour Q₁, dans laquelle Dᵢ, D₂, D₃ et D₄ représentent chacun une simple liaison, un groupe alkylène ayant de 1 à 8 atomes de carbone ou un groupe vinylène, et q1, q2, q3 et q4 représentent chacun un entier 0, 1 ou 2, ledit cycle formé avec un atome de soufre peut être encore condensé avec un cycle saturé ou non de 5 à 6 membres, à l'exception du soufre élémentaire; dans laquelle X₂ représente -COOM', -OH, -SO₃M', -CONH₂, -S0₂NH₂, -NH₂, -SH, -CN, -CO₂ R₁₆, -SO₂ R₁₆, -OR₁₆, -NR₁₆R₁₇, -SR₁₆, -SO₃ R₁₆, -NHCOR₁₆, -NHSO₂ R₁₆, -OCOR₁₆ ou -SO₂ R₁₆; Y₂ représente ou un atome d'hydrogène; et m9 et n9 représentent chacun un entier de 1 à 10; R₁₁, R₁₂, R13, R₁₄, R₁₅, R₁₇ et R₁₈ représentent chacun un atome d'hydrogène, un groupe alkyle inférieur, un groupe acyle ou
R₁₆ représente un groupe alkyle inférieur;
R₁₉ représente -NR₂₀R₂₁, -OR₂₂ ou -SR₂₂; R₂₀ et R₂₁ représentent chacun un atome d'hydrogène ou un groupe alkyle inférieur; et R₂₂ représente un groupe d'atomes nécessaire pour former un cycle en combinaison avec R₁₈; R₂₀ ou R₁₁ peuvent être combinés avec R₁₈ pour former un cycle; M' représente un atome d'hydrogène ou un cation, dans laquelle Ar représente un groupe aryle divalent ou un groupe organique divalent formé par combinaison d'un groupe aryle avec un atome d'oxygène et/ou un groupe alkylène; B₂ et B₃ représentent chacun un groupe alkylène inférieur; R₂₃, R₂₄, R₂₅ et R₂₆ représentent chacun un groupe alkyle inférieur substitué par un hydroxyle; et x et y représentent chacun 0 ou 1; G' représente un anion; et z représente 0, 1 ou 2, dans laquelle R₂₉ et R₃₀ représentent chacun un atome d'hydrogène, un groupe alkyle, un groupe aryle ou un groupe hétérocyclique; R₃, représente un atome d'hydrogène ou un groupe alkyle; R₃₂ représente un atome d'hydrogène ou un groupe carboxyle.

3. Procédé de traitement d'un matériau photographique couleur d'halogénure d'argent photosensible selon la revendication 1 ou 2, dans lequel au moins une couche dudit matériau photographique couleur d'halogénure d'argent photosensible contient un coupleur cyan de formule générale (C) : dans laquelle R₂, représente un groupe alkyle, un groupe alcényle, un groupe cycloalkyle, un groupe aryle ou un groupe hétérocyclique; R₂₄ représente un groupe aryle non substitué ou substitué; et Z représente un atome d'hydrogène ou un groupe éliminable par réaction de couplage avec un produit oxydant d'un agent développeur dérivé de p-phénylènediamine N-hydroxyalkyle substitué.

4. Procédé de traitement d'un matériau photographique couleur d'halogénure d'argent photosensible selon la revendication 1, 2 ou 3, dans lequel au moins l'un des substituants dans formule générale (M) représente un groupe sulfonyle aromatique, représenté par la formule suivante (A) : dans laquelle R représente un groupe aliphatique, un groupe aryle ou un groupe hétérocyclique; m représente un entier, 1 ou 2, R₁ peut être identique ou différent quand m est 2; R₂ représente un groupe aliphatique, un groupe aryle, un groupe hétérocyclique ou où R₃ et R₄ représentent chacun un atome d'hydrogène, un groupe aliphatique ou un groupe aryle.

5. Procédé de traitement d'un matériau photographique couleur d'halogénure d'argent photosensible selon l'une quelconque des revendications 1 à 4, dans lequel l'acide organique ou l'acide organique capable de former le complexe ferrique organique acide est un composé représenté par les formules générales suivantes (XII) ou (XIII) : dans lesquelles E représente un groupe alkylène substitué ou non substitué, un groupe cycloalkylène, un groupe phénylène, -R₈₃0R₈₃0R₈₃- ou R₈₃ZR₈₃-, Z représente N-R₈₃-A₆ ou N-A₆, R₇₉ à R₈₃ individuellement représentent un groupe alkylène substitué ou non substitué, A₂ à A₆ représentent individuellement un atome d'hydrogène, -OH, -COOM où PÛ₃M₂ et M est un atome d'hydrogène ou un atome de métal alcalin.

6. Procédé de traitement d'un matériau photographique couleur d'halogénure d'argent photosensible selon la revendication 5, dans lequel ledit composé représenté par la formule (XII) ou (XIII) est un composé choisi dans le groupe constitué de :
(XII - 1) acide éthylènediaminetétraacétique
(XII - 2) acide diéthylènetriaminepentaacétique
(XII - 4) acide propylènediaminetétraacétique
(XII - 5) acide triéthylènetétraminehexaacétique
(XII - 7) acide 1,2-diaminopropanetétraacétique
(XII - 8) acide 1,3-diaminopropane-2-ol-tétraacétique
(XII - 19) acide éthylènediaminetétraméthylène phosphonique
(XIII - 1) acide nitrilotriacétique
(XIII - 3) acide hydroxyéthyliminodiacétique
(XIII - 5) acide nitrilotriméthylène phosphonique

7. Procédé de traitement d'un matériau photographique couleur d'halogénure d'argent photosensible selon l'une quelconque des revendications 1 à 6, dans laquelle la quantité de solution de blanchiment à régénérer est de 40 ml à 250 ml par 1 m² de matériau photographique couleur d'halogénure d'argent photosensible.

8. Procédé de traitement de matériau photographique couleur d'halogénure d'argent photosensible selon la revendication 7, dans lequel la quantité de solution de blanchiment à régénérer est de 50 ml à 200 ml par 1 m² de matériau photographique couleur d'halogénure d'argent photosensible.

9. Procédé de traitement de matériau photographique couleur d'halogénure d'argent photosensible selon la revendication 2 dans lequel la solution de blanchiment contient au moins l'un des composés choisi dans le groupe constitué des composés représentés par les formules (II), (III), (V) ou (VII).

10. Procédé de traitement d'un matériau photographique couleur d'halogénure d'argent photosensible selon l'une quelconque des revendications 1 à 9, dans lequel on utilise une solution révélatrice de couleur à l'étape du développement de la couleur qui contient un agent développeur de couleur représenté par la formule suivante (X) : dans laquelle R₁₃ représente un atome d'hydrogène, un atome d'halogène, ou un groupe alkyle, ledit groupe alkyle ayant une chaîne droite ou ramifiée de 1 à 5 atomes de carbone et en option un substituant, R₁₄ et R₁₅ représentent individuellement un atome d'hydrogène, un groupe alkyle ou un groupe aryle, ledit groupe alkyle ou aryle étant substitué en variante; au moins l'un des groupes R₁₄ et R₁₅ est un groupe alkyle substitué par un groupe hydrosoluble, tel qu'un groupe hydroxy, un groupe carboxy, un groupe acide sulfonique, un groupe amino, un groupe sulfonamido ou ledit groupe alkyle étant encore substitué en variante; R₁₆ représente un atome d'hydrogène ou un groupe alkyle ayant une chaîne droite ou ramifiée de 1 à 5 atomes de carbone et p et q représentent chacun un entier de 1 à 5.

11. Procédé de traitement d'un matériau photographique couleur d'halogénure d'argent photosensible selon l'une quelconque des revendications 1 à 10 dans lequel le matériau photographique d'halogénure d'argent photosensible contient au moins l'un des composés ayant la formule générale (XI) : dans laquelle Z₁₁ et Z₂, représentent individuellement des groupes d'atomes requis pour former un cycle benzénique ou naphtalénique condensés sur un cycle oxazole; R₄₁ et R₄₂ représentent individuellement un groupe alkyle, un groupe alcényle ou un groupe aryle, R₄₃ représente un atome d'hydrogène ou un groupe alkyle ayant de 1 à 3 atomes de carbone, X₁⊖ représente un anion et n est 1 ou 0.
